



US010543402B2

(12) **United States Patent**  
Shigemitsu et al.

(10) **Patent No.:** US 10,543,402 B2  
(45) **Date of Patent:** Jan. 28, 2020

(54) **MULTI-PIECE GOLF BALL**

(71) **Applicant:** DUNLOP SPORTS CO., LTD.,  
Kobe-shi, Hyogo (JP)

(72) **Inventors:** Takahiro Shigemitsu, Kobe (JP);  
Hidetaka Inoue, Kobe (JP)

(73) **Assignee:** SUMITOMO RUBBER  
INDUSTRIES, LTD., Kobe-Shi, Hyogo  
(JP)

(\*) **Notice:** Subject to any disclaimer, the term of this  
patent is extended or adjusted under 35  
U.S.C. 154(b) by 7 days.

(21) **Appl. No.:** 14/754,288

(22) **Filed:** Jun. 29, 2015

(65) **Prior Publication Data**

US 2015/0375056 A1 Dec. 31, 2015

(30) **Foreign Application Priority Data**

Jun. 30, 2014 (JP) ..... 2014-135405  
May 14, 2015 (JP) ..... 2015-099148

(51) **Int. Cl.**

A63B 37/06 (2006.01)  
A63B 37/00 (2006.01)

(52) **U.S. Cl.**

CPC ..... A63B 37/0076 (2013.01); A63B 37/0031  
(2013.01); A63B 37/0033 (2013.01); A63B  
37/0043 (2013.01); A63B 37/0044 (2013.01);  
A63B 37/0045 (2013.01); A63B 37/0062  
(2013.01); A63B 37/0064 (2013.01); A63B  
37/0092 (2013.01)

(58) **Field of Classification Search**

CPC ..... A63B 37/0043; A63B 37/0076

USPC ..... 473/376  
See application file for complete search history.

(56) **References Cited**

**U.S. PATENT DOCUMENTS**

|                 |         |                  |       |              |
|-----------------|---------|------------------|-------|--------------|
| 6,302,808 B1 *  | 10/2001 | Dalton           | ..... | A63B 45/00   |
|                 |         |                  |       | 473/371      |
| 6,786,838 B2 *  | 9/2004  | Sullivan         | ..... | A63B 37/0003 |
|                 |         |                  |       | 473/373      |
| 7,306,528 B2 *  | 12/2007 | Jordan           | ..... | A63B 37/0003 |
|                 |         |                  |       | 473/376      |
| 2002/0034987 A1 | 3/2002  | Yamagishi et al. |       |              |

(Continued)

**FOREIGN PATENT DOCUMENTS**

|    |               |         |
|----|---------------|---------|
| JP | 8-336617 A    | 12/1996 |
| JP | 2009-233335 A | 10/2009 |

*Primary Examiner* — Raeann Gorden

(74) **Attorney, Agent, or Firm:** Birch, Stewart, Kolasch  
& Birch LLP

(57) **ABSTRACT**

An object of the present invention is to provide a golf ball showing low spin rate on driver shots and high spin rate on approach shots. The present invention provides a multi-piece golf ball comprising a spherical center, at least two envelope layers covering the spherical center, and a cover covering the envelope layers, wherein the envelope layers comprise at least a first envelope layer covering the spherical center, and a second envelope layer covering the first envelope layer, a material hardness (H0) of the spherical center, a material hardness (H1) of the first envelope layer, and a material hardness (H2) of the second envelope layer satisfy an equation of H0>H1>H2, and the material hardness (H2) of the second envelope layer is lowest among the material hardness of the center constituent material and material hardness of envelope layer constituent materials.

25 Claims, 3 Drawing Sheets



(56)

**References Cited**

U.S. PATENT DOCUMENTS

- 2004/0209706 A1\* 10/2004 Sullivan ..... A63B 37/0003  
473/371  
2007/0129172 A1\* 6/2007 Cavallaro ..... A63B 37/0003  
473/371  
2008/0261723 A1\* 10/2008 Sullivan ..... A63B 37/0003  
473/374  
2009/0011855 A1 1/2009 Sullivan et al.

\* cited by examiner



Fig. 1



Fig.2



Fig.3

## 1

## MULTI-PIECE GOLF BALL

## FIELD OF THE INVENTION

The present invention relates to a multi-piece golf ball, in particular, a multi-piece golf ball showing a low spin rate on driver shots and a high spin rate on approach shots.

## DESCRIPTION OF THE RELATED ART

As a method of inhibiting the spin rate on driver shots, a method of controlling the hardness distribution of the golf ball is exemplified. For example, by adopting an outer-hard and inner-soft hardness distribution in the golf ball, the spin rate on driver shots can be lowered, thus the flight distance on driver shots can be increased.

As the golf ball having a controlled hardness distribution, for example, Japanese Patent Publication No. H08-336617 A discloses a multi-piece solid golf ball having a structure of at least four layers consisting of a core having a structure of at least two layers and two cover layers covering the core, wherein the outer cover has a hardness of 40 to 60 in Shore D hardness, and the inner cover has a hardness of 53 or less in Shore D hardness and lower than the hardness of the outer cover.

Japanese Patent Publication No. 2009-233335 A discloses a golf ball including: a unitary core having a volume, an outer surface, a geometric center, and an outermost transition part adjacent to the outer surface, the core being formed from a substantially homogenous composition; and a cover layer, wherein the outermost transition part is disposed between the core outer surface and the geometric center, the transition part has an outer portion congruent with the core outer surface and comprises the outermost 45% of the core volume or less, and both a hardness of the core outer surface and a hardness within the outermost transition part are less than a hardness of the geometric center to define a negative hardness gradient.

## SUMMARY OF THE INVENTION

By adopting the outer-hard and inner-soft hardness distribution in the golf ball, the spin rate on driver shots can be lowered. However, in this case, not only the spin rate on driver shots is lowered, but also the spin rate on approach shots tends to be lowered. Therefore, although the golf ball having the outer-hard and inner-soft structure shows an improved flight distance on driver shots, its controllability on approach shots tends to be lowered.

The present invention has been achieved in view of the above problems. An object of the present invention is to provide a multi-piece golf ball showing a low spin rate on driver shots and a high spin rate on approach shots.

The present invention provide a multi-piece golf ball comprising a spherical center, at least two envelope layers covering the spherical center, and a cover covering the envelope layers, wherein the envelope layers comprise at least a first envelope layer covering the spherical center, and a second envelope layer covering the first envelope layer, a material hardness (H0) of the spherical center, a material hardness (H1) of the first envelope layer, and a material hardness (H2) of the second envelope layer satisfy an equation of  $H0 > H1 > H2$ , and the material hardness (H2) of the second envelope layer is lowest among the material hardness of the center constituent material and the material hardness of the envelope layer constituent material. By constituted as above, the multi-piece golf ball of the present

## 2

invention has an appropriate hardness distribution. By having the appropriate hardness distribution, the spin rate on driver shots is lowered, and the spin rate on approach shots becomes higher.

According to the present invention, a multi-piece golf ball showing a low spin rate on driver shots and a high spin rate on approach shots can be obtained.

## BRIEF DESCRIPTION OF THE DRAWINGS

10 FIG. 1 is a schematic sectional view showing one example of a structure of a golf ball according to the present invention.

15 FIG. 2 is a schematic sectional view showing another example of a structure of a golf ball according to the present invention.

20 FIG. 3 is a partially cutaway view of a golf ball of one embodiment according to the present invention.

## DESCRIPTION OF THE PREFERRED EMBODIMENT

25 The present invention provides a multi-piece golf ball comprising a spherical center, at least two envelope layers covering the spherical center, and a cover covering the envelope layers, wherein the envelope layers comprise at least a first envelope layer covering the spherical center, and a second envelope layer covering the first envelope layer, a material hardness (H0) of the spherical center, a material hardness (H1) of the first envelope layer, and a material hardness (H2) of the second envelope layer satisfy an equation of  $H0 > H1 > H2$ , and the material hardness (H2) of the second envelope layer is lowest among the material hardness of the center constituent material and material hardness of envelope layer constituent materials.

## 30 (1) Structure of Golf Ball

35 In the follows, the present invention will be described with reference to drawings. FIG. 1 is a schematic sectional view showing a structure of a multi-piece golf ball according to the present invention. The multi-piece golf ball according to the present invention comprises a spherical center Ce, at least two envelope layers covering the spherical center, and a cover Co covering the envelope layers, and the envelope layers comprise at least a first envelope layer E1 directly covering the spherical center, and a second envelope layer E2 directly covering the first envelope layer. The envelope layers preferably comprise at least three layers and more preferably comprise at least four layers, and preferably comprise at most ten layers and more preferably comprise at most nine layers. If the envelope layers comprise at least three layers, it becomes easier to control the hardness distribution of the golf ball. On the other hand, if the number of the envelope layers is excessively large, the moldability of the envelope layers is lowered. It is noted that a paint film and a reinforcement layer (adhesive agent layer) that is provided to improve adhesion between the envelope layers are not included in the envelope layers. The paint film and the reinforcement layer (adhesive agent layer) have a different film thickness range from the envelope layers. The paint film and the reinforcement layer (adhesive agent layer) generally have a film thickness of 50  $\mu\text{m}$  (0.050 mm) or less.

40 In the multi-piece golf ball, the material hardness (H1) (Shore D hardness) of the first envelope layer is lower than the material hardness (H0) (Shore D hardness) of the center (H0 > H1). The hardness difference (H0 - H1) between the hardness (H1) and the hardness (H0) is preferably 1 or more, more preferably 1.5 or more, and even more preferably 2 or

more, and is preferably 30 or less, more preferably 25 or less, and even more preferably 20 or less in Shore D hardness. If the hardness difference (H0-H1) falls within the above range, the spin rate on driver shots is further lowered.

The hardness (Shore D hardness) ratio (H0/H1) between the hardness (H1) and the hardness (H0) is preferably 1.01 or more, more preferably 1.02 or more, and even more preferably 1.05 or more, and is preferably 3.0 or less, more preferably 2.9 or less, and even more preferably 2.8 or less. If the hardness ratio (H0/H1) is 1.01 or more, the spin rate on driver shots is further lowered, and if the hardness ratio (H0/H1) is 3.0 or less, the resilience of the golf ball becomes better.

In the multi-piece golf ball, the material hardness (H2) (Shore D hardness) of the second envelope layer is lower than the material hardness (H1) (Shore D hardness) of the first envelope layer (H1>H2). The hardness difference (H1-H2) between the hardness (H2) and the hardness (H1) is preferably 1 or more, more preferably 1.5 or more, and even more preferably 2 or more, and is preferably 30 or less, more preferably 25 or less, and even more preferably 20 or less in Shore D hardness. If the hardness difference (H1-H2) falls within the above range, the spin rate on driver shots is further lowered.

The hardness (Shore D hardness) ratio (H1/H2) between the hardness (H2) and the hardness (H1) is preferably 1.01 or more, more preferably 1.02 or more, and even more preferably 1.05 or more, and is preferably 3.0 or less, more preferably 2.9 or less, and even more preferably 2.8 or less. If the hardness ratio (H1/H2) is 1.01 or more, the spin rate on driver shots is further lowered, and if the hardness ratio (H1/H2) is 3.0 or less, the resilience of the golf ball becomes better.

The hardness difference (H0-H2) between the hardness (H2) and the hardness (H0) is preferably 1 or more, more preferably 2 or more, and even more preferably 3 or more, and is preferably 50 or less, more preferably 45 or less, and even more preferably 40 or less in Shore D hardness. If the hardness difference (H0-H2) is 1 or more in Shore D hardness, the spin rate on driver shots is effectively lowered, and if the hardness difference (H0-H2) is 50 or less in Shore D hardness, the durability of the golf ball is sufficiently maintained.

The hardness (Shore D hardness) ratio (H0/H2) between the hardness (H2) and the hardness (H0) is preferably 1.05 or more, more preferably 1.10 or more, and even more preferably 1.15 or more, and is preferably 30 or less, more preferably 20 or less, and even more preferably 10 or less. If the hardness ratio (H0/H2) is 1.05 or more, the spin rate on driver shots is effectively lowered, and if the hardness ratio (H0/H2) is 30 or less, the durability of the golf ball is sufficiently maintained.

The material hardness (H2) of the second envelope layer is lowest among the material hardness of the center constituent material and material hardness of the envelope layer constituent materials. By making the material hardness of the second envelope layer lowest, the spin rate on driver shots is further lowered. The material hardness (H2) is preferably 2 or more, more preferably 3 or more, and even more preferably 5 or more, and is preferably 30 or less, more preferably 27 or less, and even more preferably 25 or less in Shore D hardness. If the material hardness (H2) is 2 or more, the resilience of the golf ball is not lowered, and if the material hardness (H2) is 30 or less, the spin rate on driver shots is effectively lowered. It is also preferable that the

material hardness (H2) of the second envelope layer is lowest among the material hardness of the golf ball constituent materials.

The material hardness (H1) is preferably 10 or more, more preferably 15 or more, and even more preferably 20 or more, and is preferably 50 or less, more preferably 45 or less, and even more preferably 40 or less in Shore D hardness. If the material hardness (H1) is 10 or more, the resilience of the golf ball becomes better, and if the material hardness (H1) is 50 or less, the spin rate on driver shots is further lowered.

The material hardness (H0) is preferably 15 or more, more preferably 20 or more, even more preferably 25 or more, and mostly preferably 30 or more, and is preferably 55 or less, more preferably 50 or less, and even more preferably 45 or less in Shore D hardness. If the material hardness (H0) falls within the above range, the resilience of the golf ball is not lowered.

The diameter of the spherical center is preferably 5 mm or more, more preferably 7 mm or more, and even more preferably 10 mm or more, and is preferably 25 mm or less, more preferably 22 mm or less, and even more preferably 15 mm or less. If the diameter of the spherical center is 5 mm or more, the spin rate on driver shots is further lowered. On the other hand, if the diameter of the spherical center is 25 mm or less, the spin rate on approach shots is hardly lowered.

When the center has a diameter in a range from 5 mm to 25 mm, the compression deformation amount (shrinking amount of the center along the compression direction) of the center when applying a load from 98 N as an initial load to 1275 N as a final load to the center is preferably 1.5 mm or more, more preferably 1.7 mm or more, and even more preferably 2.0 mm or more, and is preferably 5.0 mm or less, more preferably 4.7 mm or less, and even more preferably 4.5 mm or less. If the compression deformation amount is 1.5 mm or more, the shot feeling becomes better, while if the compression deformation amount is 5.0 mm or less, the resilience of the golf ball becomes better.

The thickness of the first envelope layer (E1) is preferably 0.1 mm or more, more preferably 0.2 mm or more, and even more preferably 0.3 mm or more, and is preferably 15 mm or less, more preferably 13 mm or less, and even more preferably 10 mm or less. If the thickness of the first envelope layer (E1) is 0.1 mm or more, the spin rate on driver shots is effectively lowered, and if the thickness of the first envelope layer (E1) is 15 mm or less, the resilience of the golf ball is not lowered.

The thickness of the second envelope layer (E2) is preferably 0.2 mm or more, more preferably 0.5 mm or more, and even more preferably 1.0 mm or more, and is preferably 20 mm or less, more preferably 17 mm or less, and even more preferably 15 mm or less. If the thickness of the second envelope layer (E2) is 0.2 mm or more, the spin rate on driver shots is effectively lowered, and if the thickness of the second envelope layer (E2) is 20 mm or less, the resilience of the golf ball is not lowered.

FIG. 2 is a schematic sectional view showing another structure of a multi-piece golf ball according to the present invention. As shown in FIG. 2, it is preferable that the multi-piece golf ball according to the present invention comprises a spherical center Ce, at least three envelope layers covering the spherical center, and a cover Co covering the envelope layers, and the envelope layers comprise at least a first envelope layer E1 covering the spherical center, a second envelope layer E2 covering the first envelope layer, and an outermost envelope layer En disposed on the outer side of the second envelope layer. In the case that the

envelope layers comprise at least three layers, it is preferable that the material hardness (Hn) of the outermost envelope layer En locating on the outermost side among these envelope layers is highest among the material hardness of the golf ball constituent materials. By making the material hardness of the outermost envelope layer highest, decrease of the spin rate on approach shots can be suppressed.

The material hardness (Hn) is preferably 30 or more, more preferably 35 or more, and even more preferably 40 or more, and is preferably 85 or less, more preferably 80 or less, and even more preferably 77 or less in Shore D hardness. If the material hardness (Hn) is 30 or more, the spin rate on driver shots is lowered, and if the material hardness (Hn) is 85 or less, the shot feeling becomes better.

The hardness difference (Hn-H0) between the hardness (Hn) and the hardness (H0) is preferably 1 or more, more preferably 5 or more, and even more preferably 10 or more, and is preferably 70 or less, more preferably 65 or less, and even more preferably 60 or less in Shore D hardness. If the hardness difference (Hn-H0) is 1 or more in Shore D hardness, the spin rate on driver shots is effectively lowered, and if the hardness difference (Hn-H0) is 70 or less in Shore D hardness, the resilience of the golf ball is not lowered.

The hardness (Shore D hardness) ratio (Hn/H0) between the hardness (Hn) and the hardness (H0) is preferably 1.0 or more, more preferably 1.1 or more, and even more preferably 1.2 or more, and is preferably 45 or less, and more preferably 40 or less. If the hardness ratio (Hn/H0) is 1.0 or more, the spin rate on driver shots is effectively lowered, and if the hardness ratio (Hn/H0) is 45 or less, the durability of the golf ball is sufficiently maintained.

The hardness difference (Hn-H2) between the hardness (Hn) and the hardness (H2) is preferably 25 or more, more preferably 30 or more, and even more preferably 32 or more, most preferably 34 or more, and is preferably 80 or less, more preferably 75 or less, and even more preferably 70 or less in Shore D hardness. If the hardness difference (Hn-H2) is 30 or more in Shore D hardness, the spin rate on driver shots is effectively lowered, and if the hardness difference (Hn-H2) is 80 or less in Shore D hardness, the shot feeling becomes better.

The hardness (Shore D hardness) ratio (Hn/H2) between the hardness (Hn) and the hardness (H2) is preferably 1.05 or more, more preferably 1.10 or more, and even more preferably 1.15 or more, and is preferably 30 or less, more preferably 20 or less, and even more preferably 10 or less. If the hardness ratio (Hn/H2) is 1.05 or more, the spin rate on driver shots is effectively lowered, and if the hardness ratio (Hn/H2) is 30 or less, the durability of the golf ball is sufficiently maintained.

The thickness of the outermost envelope layer (En) is preferably 0.1 mm or more, more preferably 0.2 mm or more, and even more preferably 0.5 mm or more, and is preferably 5 mm or less, more preferably 4 mm or less, and even more preferably 3 mm or less. If the thickness of the outermost envelope layer (En) is 0.1 mm or more, the durability of the golf ball is sufficiently maintained, and if the thickness of the outermost envelope layer (En) is 5 mm or less, the shot feeling becomes better.

When another envelope layer is disposed between the second envelope layer (E2) and the outermost envelope layer (En), the hardness (Hx) of the material forming another envelope layer is preferably higher than the hardness (H2) and smaller than the hardness (Hn) ( $H2 < Hx < Hn$ ).

The thickness of another envelope layer is not particularly limited, but the thickness of another envelope layer is preferably 0.1 mm or more, more preferably 0.2 mm or

more, and even more preferably 0.3 mm or more, and is preferably 15 mm or less, more preferably 13 mm or less, and even more preferably 10 mm or less.

The material hardness (Hc) of the cover is preferably 5 or more, more preferably 7 or more, and even more preferably 10 or more, and is preferably 55 or less, more preferably 53 or less, and even more preferably 50 or less in Shore D hardness. If the material hardness (Hc) of the cover falls within the above range, the spin rate on approach shots is further increased.

The thickness of the cover is preferably 2.0 mm or less, more preferably 1.6 mm or less, even more preferably 1.2 mm or less, and mostly preferably 1.0 mm or less. If the thickness of the cover is 2.0 mm or less, the resilience and shot feeling of the obtained golf ball become better. The thickness of the cover is preferably 0.1 mm or more, more preferably 0.2 mm or more, and even more preferably 0.3 mm or more. If the thickness of the cover is less than 0.1 mm, molding the cover may become difficult, and the durability and wear resistance of the cover may deteriorate.

The multi-piece golf ball preferably has a diameter ranging from 40 mm to 45 mm. In light of satisfying the regulation of US Golf Association (USGA), the diameter is mostly preferably 42.67 mm or more. In light of prevention of air resistance, the diameter is more preferably 44 mm or less, and mostly preferably 42.80 mm or less. In addition, the multi-piece golf ball preferably has a mass of 40 g or more and 50 g or less. In light of obtaining greater inertia, the mass is more preferably 44 g or more, and mostly preferably 45.00 g or more. In light of satisfying the regulation of USGA, the mass is mostly preferably 45.93 g or less.

When the multi-piece golf ball has a diameter in a range from 40 mm to 45 mm, the compression deformation amount (shrinking amount along the compression direction) of the multi-piece golf ball when applying a load from 98 N as an initial load to 1275 N as a final load to the multi-piece golf ball is preferably 2.0 mm or more and more preferably 2.2 mm or more, and is preferably 4.0 mm or less and more preferably 3.5 mm or less. If the compression deformation amount is 2.0 mm or more, the golf ball does not become excessively hard, so the shot feeling thereof becomes better. On the other hand, if the compression deformation amount is 4.0 mm or less, the resilience of the golf ball becomes better.

#### 45 (2) Golf Ball Constituent Material

The constituent materials constituting the multi-piece golf ball according to the present invention will be described. The constituent materials constituting the multi-piece golf ball according to the present invention are a thermoplastic resin composition and a rubber composition forming the center, the envelope layers or the cover. The material hardness of each material can be adjusted by changing the material formulation.

#### Thermoplastic Resin Composition

55 Firstly, the thermoplastic resin composition used in the present invention will be explained. (A) The resin component contained in the thermoplastic resin composition is not particularly limited, as long as it is a thermoplastic resin. Examples of the thermoplastic resin include, for example, a thermoplastic resin such as an ionomer resin, a thermoplastic olefin copolymer, a thermoplastic polyurethane resin, a thermoplastic polyamide resin, a thermoplastic styrene-based resin, a thermoplastic polyester resin, a thermoplastic acrylic resin, and the like. Among these thermoplastic resins, a thermoplastic elastomer having rubber elasticity is preferable. Examples of the thermoplastic elastomer include, for example, a thermoplastic polyurethane elastomer, a thermo-

plastic polyamide elastomer, a thermoplastic styrene-based elastomer, a thermoplastic polyester elastomer, a thermoplastic acrylic-based elastomer, and the like.

(2-1) Ionomer Resin

Examples of the ionomer resin include: an ionomer resin consisting of a metal ion-neutralized product of a binary copolymer composed of an olefin and an  $\alpha,\beta$ -unsaturated carboxylic acid having 3 to 8 carbon atoms; an ionomer resin consisting of a metal ion-neutralized product of a ternary copolymer composed of an olefin, an  $\alpha,\beta$ -unsaturated carboxylic acid having 3 to 8 carbon atoms and an  $\alpha,\beta$ -unsaturated carboxylic acid ester; or a mixture thereof.

In the present invention, "the ionomer resin consisting of a metal ion-neutralized product of a binary copolymer composed of an olefin and an  $\alpha,\beta$ -unsaturated carboxylic acid having 3 to 8 carbon atoms" is sometimes merely referred to as "the binary ionomer resin", and "the ionomer resin consisting of a metal ion-neutralized product of a ternary copolymer composed of an olefin, an  $\alpha,\beta$ -unsaturated carboxylic acid having 3 to 8 carbon atoms and an  $\alpha,\beta$ -unsaturated carboxylic acid ester" is sometimes merely referred to as "the ternary ionomer resin".

The olefin is preferably an olefin having 2 to 8 carbon atoms. Examples of the olefin include, for example, ethylene, propylene, butene, pentene, hexene, heptane and octane, and ethylene is particularly preferred. Examples of the  $\alpha,\beta$ -unsaturated carboxylic acid having 3 to 8 carbon atoms include, for example, acrylic acid, methacrylic acid, fumaric acid, maleic acid and crotonic acid, and acrylic acid and methacrylic acid are particularly preferred. In addition, examples of the  $\alpha,\beta$ -unsaturated carboxylic acid ester include, for example, methyl ester, ethyl ester, propyl ester, n-butyl ester, isobutyl ester of acrylic acid, methacrylic acid, fumaric acid and maleic acid, and acrylic acid ester and methacrylic acid ester are particularly preferred.

The binary ionomer resin is preferably a metal ion-neutralized product of a binary copolymer composed of ethylene-(meth)acrylic acid. The ternary ionomer resin is preferably a metal ion-neutralized product of a ternary copolymer composed of ethylene, (meth)acrylic acid and (meth)acrylic acid ester. Here, (meth)acrylic acid means acrylic acid and/or methacrylic acid.

The content of the  $\alpha,\beta$ -unsaturated carboxylic acid component having 3 to 8 carbon atoms in the binary ionomer resin is preferably 15 mass % or more, more preferably 16 mass % or more, and even more preferably 17 mass % or more, and is preferably 30 mass % or less, more preferably 25 mass % or less. If the content of the  $\alpha,\beta$ -unsaturated carboxylic acid component having 3 to 8 carbon atoms is 15 mass % or more, the resultant constituent member has a desirable hardness. If the content of the  $\alpha,\beta$ -unsaturated carboxylic acid component having 3 to 8 carbon atoms is 30 mass % or less, since the hardness of the resultant constituent member does not become excessively high, the durability and the shot feeling thereof become better.

The degree of neutralization of the carboxyl groups of the binary ionomer resin is preferably 15 mole % or more, more preferably 20 mole % or more, and is preferably 100 mole % or less. If the degree of neutralization is 15 mole % or more, the resultant golf ball has better resilience and durability. The degree of neutralization of the carboxyl groups of the binary ionomer resin can be calculated by the following expression. Sometimes, the metal component is contained in such an amount that the theoretical degree of neutralization of the carboxyl groups contained in the ionomer resin exceeds 100 mole %.

Degree of neutralization (mole %) of the binary ionomer resin=100 $\times$  the number of moles of carboxyl groups neutralized in the binary ionomer resin/the number of moles of all carboxyl groups contained in the binary ionomer resin

5 Examples of the metal ion used for neutralizing at least a part of carboxyl groups of the binary ionomer resin include: a monovalent metal ion such as sodium, potassium, lithium; a divalent metal ion such as magnesium, calcium, zinc, barium, cadmium; a trivalent metal ion such as aluminum; 10 and other ion such as tin, zirconium.

Specific examples of the binary ionomer resin include trade name "Himilan (registered trademark) (e.g. Himilan 1555 (Na), Himilan 1557 (Zn), Himilan 1605 (Na), Himilan 1706 (Zn), Himilan 1707 (Na), Himilan AM7311 (Mg), 15 Himilan AM7329 (Zn))" commercially available from Mitsui-Du Pont Polymers Co., Ltd.

Further, examples include "Surlyn (registered trademark) (e.g. Surlyn 8945 (Na), Surlyn 9945 (Zn), Surlyn 8140 (Na), Surlyn 8150 (Na), Surlyn 9120 (Zn), Surlyn 9150 (Zn), 20 Surlyn 6910 (Mg), Surlyn 6120 (Mg), Surlyn 7930 (Li), Surlyn 7940 (Li), Surlyn AD8546 (Li))" commercially available from E.I. du Pont de Nemours and Company.

Further, examples include "Iotek (registered trademark) (e.g. Iotek 8000 (Na), Iotek 8030 (Na), Iotek 7010 (Zn), 25 Iotek 7030 (Zn))" commercially available from ExxonMobil Chemical Corporation.

The binary ionomer resins may be used alone or as a mixture of at least two of them. It is noted that Na, Zn, Li and Mg described in the parentheses after the trade names 30 indicate metal types of neutralizing metal ions of the binary ionomer resins.

The binary ionomer resin preferably has a bending stiffness of 140 MPa or more, more preferably 150 MPa or more, and even more preferably 160 MPa or more, and preferably 35 has a bending stiffness of 550 MPa or less, more preferably 500 MPa or less, even more preferably 450 MPa or less. If the bending stiffness of the binary ionomer resin is excessively low, the flight distance tends to be shorter because of the increased spin rate of the golf ball. If the bending 40 stiffness is excessively high, the durability of the golf ball may be lowered.

The binary ionomer resin preferably has a melt flow rate (190° C., 2.16 kgf) of 0.1 g/10 min or more, more preferably 45 0.5 g/10 min or more, even more preferably 1.0 g/10 min or more, and preferably has a melt flow rate (190° C., 2.16 kgf) of 30 g/10 min or less, more preferably 20 g/10 min or less, even more preferably 15 g/10 min or less. If the melt flow rate (190° C., 2.16 kgf) of the binary ionomer resin is 0.1 g/10 min or more, the thermoplastic resin composition has better fluidity, thus, for example, molding a thin layer becomes possible. If the melt flow rate (190° C., 2.16 kgf) of the binary ionomer resin is 30 g/10 min or less, the durability of the resultant golf ball becomes better.

The content of the  $\alpha,\beta$ -unsaturated carboxylic acid component having 3 to 8 carbon atoms in the ternary ionomer resin is preferably 2 mass % or more, more preferably 3 mass % or more, and is preferably 30 mass % or less, more 55 preferably 25 mass % or less.

The degree of neutralization of the carboxyl groups of the 60 ternary ionomer resin is preferably 20 mole % or more, more preferably 30 mole % or more, and is preferably 100 mole % or less. If the degree of neutralization is 20 mole % or more, the resultant golf ball obtained by using the thermoplastic resin composition has better resilience and durability.

65 The degree of neutralization of the carboxyl groups of the ionomer resin can be calculated by the following expression. Sometimes, the metal component is contained in such an

amount that the theoretical degree of neutralization of the carboxyl groups of the ionomer resin exceeds 100 mole %.

Degree of neutralization (mole %) of the ionomer resin=100 $\times$  the number of moles of carboxyl groups neutralized in the ionomer resin/the number of moles of all carboxyl groups contained in the ionomer resin

Examples of the metal ion used for neutralizing at least a part of carboxyl groups of the ternary ionomer resin include: a monovalent metal ion such as sodium, potassium, lithium; a divalent metal ion such as magnesium, calcium, zinc, barium, cadmium; a trivalent metal ion such as aluminum; and other ion such as tin, zirconium.

Specific examples of the ternary ionomer resin include trade name "Himilan (registered trademark) (e.g. Himilan AM7327 (Zn), Himilan 1855 (Zn), Himilan 1856 (Na), Himilan AM7331 (Na))" commercially available from Mitsui-Du Pont Polymers Co., Ltd. Further, the ternary ionomer resins commercially available from E.I. du Pont de Nemours and Company include "Surlyn 6320 (Mg), Surlyn 8120 (Na), Surlyn 8320 (Na), Surlyn 9320 (Zn), Surlyn 9320W (Zn), HPF1000 (Mg), HPF2000 (Mg) or the like". The ternary ionomer resins commercially available from ExxonMobil Chemical Corporation include "Iotek 7510 (Zn), Iotek 7520 (Zn) or the like". It is noted that Na, Zn and Mg described in the parentheses after the trade names indicate metal types of neutralizing metal ions. The ternary ionomer resins may be used alone or as a mixture of at least two of them.

The ternary ionomer resin preferably has a bending stiffness of 10 MPa or more, more preferably 11 MPa or more, even more preferably 12 MPa or more, and preferably has a bending stiffness of 100 MPa or less, more preferably 97 MPa or less, even more preferably 95 MPa or less. If the bending stiffness of the ternary ionomer resin is excessively low, the flight distance tends to be shorter because of the increased spin rate of the golf ball. If the bending stiffness is excessively high, the durability of the golf ball may be lowered.

The ternary ionomer resin preferably has a melt flow rate (190° C., 2.16 kgf) of 0.1 g/10 min or more, more preferably 0.3 g/10 min or more, even more preferably 0.5 g/10 min or more, and preferably has a melt flow rate (190° C., 2.16 kgf) of 20 g/10 min or less, more preferably 15 g/10 min or less, even more preferably 10 g/10 min or less. If the melt flow rate (190° C., 2.16 kgf) of the ternary ionomer resin is 0.1 g/10 min or more, the thermoplastic resin composition has better fluidity, thus it is easy to mold a thin envelope layer. If the melt flow rate (190° C., 2.16 kgf) of the ternary ionomer resin is 20 g/10 min or less, the durability of the resultant golf ball becomes better.

The ternary ionomer resin preferably has a slab hardness of 20 or more, more preferably 25 or more, even more preferably 30 or more, and preferably has a slab hardness of 70 or less, more preferably 65 or less, even more preferably 60 or less in Shore D hardness. If the ternary ionomer resin has a slab hardness of 20 or more in Shore D hardness, the resultant constituent member does not become excessively soft and thus the golf ball has better resilience. If the ternary ionomer resin has a slab hardness of 70 or less in Shore D hardness, the resultant constituent member does not become excessively hard and thus the golf ball has better durability.

#### (2-2) Thermoplastic Olefin Copolymer

Examples of the thermoplastic olefin copolymer include, for example, a binary copolymer composed of an olefin and an  $\alpha,\beta$ -unsaturated carboxylic acid having 3 to 8 carbon atoms; a ternary copolymer composed of an olefin, an  $\alpha,\beta$ -unsaturated carboxylic acid having 3 to 8 carbon atoms,

and an  $\alpha,\beta$ -unsaturated carboxylic acid ester; or a mixture thereof. The thermoplastic olefin copolymer is a nonionic copolymer in which the carboxyl groups are not neutralized.

In the present invention, "the binary copolymer composed of an olefin and an  $\alpha,\beta$ -unsaturated carboxylic acid having 3 to 8 carbon atoms" is sometimes merely referred to as "the binary copolymer", and the ternary copolymer composed of an olefin, an  $\alpha,\beta$ -unsaturated carboxylic acid having 3 to 8 carbon atoms, and an  $\alpha,\beta$ -unsaturated carboxylic acid ester" is sometimes merely referred to as "the ternary copolymer".

Examples of the olefin include the same as the olefin constituting the ionomer resin, and ethylene is particularly preferred. Examples of the  $\alpha,\beta$ -unsaturated carboxylic acid having 3 to 8 carbon atoms and the ester include the same as the  $\alpha,\beta$ -unsaturated carboxylic acid having 3 to 8 carbon atoms and the ester constituting the ionomer resin.

The binary copolymer is preferably a binary copolymer composed of ethylene and (meth)acrylic acid. The ternary copolymer is preferably a ternary copolymer composed of ethylene, (meth)acrylic acid, and (meth)acrylic acid ester. Here, (meth)acrylic acid means acrylic acid and/or methacrylic acid.

The content of the  $\alpha,\beta$ -unsaturated carboxylic acid having 3 to 8 carbon atoms in the binary copolymer or the ternary copolymer is preferably 4 mass % or more, more preferably 5 mass % or more, and is preferably 30 mass % or less, more preferably 25 mass % or less.

The binary copolymer or the ternary copolymer preferably has a melt flow rate (190° C., 2.16 kgf) of 5 g/10 min or more, more preferably 10 g/10 min or more, even more preferably 15 g/10 min or more, and preferably has a melt flow rate (190° C., 2.16 kgf) of 1,700 g/10 min or less, more preferably 1,500 g/10 min or less, even more preferably 1,300 g/10 min or less. If the melt flow rate (190° C., 2.16 kgf) of the binary copolymer or the ternary copolymer is 5 g/10 min or more, the thermoplastic resin composition has better fluidity and thus it is easy to mold a constituent member. If the melt flow rate (190° C., 2.16 kgf) of the binary copolymer or the ternary copolymer is 1,700 g/10 min or less, the resultant golf ball has better durability.

Specific examples of the binary copolymer include: an ethylene-methacrylic acid copolymer having a trade name of "NUCREL (registered trademark) (e.g. "NUCREL N1050H", "NUCREL N2050H", "NUCREL N110H", "NUCREL NO200H")" commercially available from Mitsui-Du Pont Polymers Co., Ltd; an ethylene-acrylic acid copolymer having a trade name of "PRIMACOR (registered trademark) 59801" commercially available from Dow Chemical Company; and the like.

Specific examples of the ternary copolymer include: the ternary copolymer having a trade name of "NUCREL (registered trademark) (e.g. "NUCREL AN4318", "NUCREL AN4319")" commercially available from Mitsui-Du Pont Polymers Co., Ltd; the ternary copolymer having a trade name of "NUCREL (registered trademark) (e.g. "NUCREL AE")" commercially available from E.I. du Pont de Nemours and Company; the ternary copolymer having a trade name of "PRIMACOR (registered trademark) (e.g. "PRIMACOR AT310", "PRIMACOR AT320")" commercially available from Dow Chemical Company; and the like. The binary copolymer or the ternary copolymer may be used alone or as a mixture of at least two of them.

#### (2-3) Thermoplastic Polyurethane Resin and Thermoplastic Polyurethane Elastomer

Examples of the thermoplastic polyurethane resin and the thermoplastic polyurethane elastomer include a thermoplastic resin and a thermoplastic elastomer which have plurality

of urethane bonds in the main molecular chain. The polyurethane is preferably a product obtained by a reaction between a polyisocyanate component and a polyol component. Examples of the thermoplastic polyurethane elastomer include, for example, trade names of "Elastollan XNY85A", "Elastollan XNY90A", "Elastollan XNY97A", "Elastollan ET885", and "Elastollan ET890" manufactured by BASF Japan Ltd and the like.

(2-4) Thermoplastic Styrene-Based Elastomer

A thermoplastic elastomer containing a styrene block can be appropriately used as the thermoplastic styrene-based elastomer. The thermoplastic elastomer containing a styrene block has a polystyrene block which is a hard segment, and a soft segment. Typical soft segment is a diene block. Examples of a constituent component of the diene block include butadiene, isoprene, 1,3-pentadiene and 2,3-dimethyl-1,3-butadiene. Butadiene and isoprene are preferable. Two or more constituent components may be used in combination.

The thermoplastic elastomer containing a styrene block includes: a styrene-butadiene-styrene block copolymer (SBS), a styrene-isoprene-styrene block copolymer (SIS), a styrene-isoprene-butadiene-styrene block copolymer (SIBS), a hydrogenated product of SBS, a hydrogenated product of SIS and a hydrogenated product of SIBS. Examples of the hydrogenated product of SBS include a styrene-ethylene-butylene-styrene block copolymer (SEBS). Examples of the hydrogenated product of SIS include a styrene-ethylene-propylene-styrene block copolymer (SEPS). Examples of the hydrogenated product of SIBS include a styrene-ethylene-ethylene-propylene-styrene block copolymer (SEEPS).

The content of the styrene component in the thermoplastic elastomer containing a styrene block is preferably 10 mass % or more, more preferably 12 mass % or more, even more preferably 15 mass % or more. In the view of the shot feeling of the resultant golf ball, the content is preferably 50 mass % or less, more preferably 47 mass % or less, even more preferably 45 mass % or less.

The thermoplastic elastomer containing a styrene block includes an alloy of one kind or two or more kinds selected from the group consisting of SBS, SIS, SIBS, SEBS, SEPS, SEEPS and a hydrogenated product thereof with a polyolefin. It is estimated that the olefin component in the alloy contributes to the improvement in compatibility with the ionomer resin. By using the alloy, the resilience of the golf ball is increased. An olefin having 2 to 10 carbon atoms is preferably used. Appropriate examples of the olefin include ethylene, propylene, butane and pentene. Ethylene and propylene are particularly preferred.

Specific examples of the polymer alloy include the polymer alloys having trade names of "Rabalon T3221C", "Rabalon T3339C", "Rabalon SJ4400N", "Rabalon SJ5400N", "Rabalon SJ6400N", "Rabalon SJ7400N", "Rabalon SJ8400N", "Rabalon SJ9400N" and "Rabalon SR04" manufactured by Mitsubishi Chemical Corporation. Other specific examples of the thermoplastic elastomer containing a styrene block include "Epofriend A1010" manufactured by Daicel Chemical Industries, Ltd and "Septon HG-252" manufactured by Kuraray Co., Ltd.

(2-5) Thermoplastic Polyamide Resin and Thermoplastic Polyamide Elastomer

The thermoplastic polyamide is not particularly limited, as long as it is a thermoplastic resin having plurality of amide bonds (—NH—CO—) in the main molecular chain. Examples of the thermoplastic polyamide include, for example, a product having an amide bond in the molecule

formed by a ring-opening polymerization of lactam or a reaction between a diamine component and a dicarboxylic acid component.

Examples of the polyamide resin include, for example, an aliphatic polyamide such as polyamide 6, polyamide 11, polyamide 12, polyamide 66, polyamide 610, polyamide 6T, polyamide 61, polyamide 9T, polyamide MST, polyamide 612; and an aromatic polyamide such as poly-p-phenylene-terephthalamide, poly-m-phenyleneisophthalamide. These polyamides may be used alone or in combination of at least two of them. Among them, the aliphatic polyamide such as polyamide 6, polyamide 66, polyamide 11, polyamide 12 is preferable.

Specific examples of the polyamide resin include, for example, the polyamide resin having a trade name of "Rilsan (registered trademark) B" (e.g. Rilsan BESN TL, Rilsan BESN P20 TL, Rilsan BESN P40 TL, Rilsan MB3610, Rilsan BMF O, Rilsan BMN O, Rilsan BMN O TLD, Rilsan BMN BK TLD, Rilsan BMN P20 D, Rilsan BMN P40 D and the like)" commercially available from Arkema Inc., and the like.

The polyamide elastomer has a hard segment part consisting of a polyamide component and a soft segment part. Examples of the soft segment part of the polyamide elastomer include, for example, a polyether ester component or a polyether component. Examples of the polyamide elastomer include, for example, a polyether ester amide obtained by a reaction between a polyamide component (hard segment component) and a polyether ester component (soft segment component) consisting of polyoxyalkylene glycol and dicarboxylic acid; and a polyether amide obtained by a reaction between a polyamide component (hard segment component) and a polyether (soft segment component) consisting of a product obtained by aminating or carboxylating two terminal ends of polyoxyalkylene glycol and dicarboxylic acid or diamine.

Examples of the polyamide elastomer include, for example, "Pebax 2533", "Pebax 3533", "Pebax 4033", "Pebax 5533" manufactured by Arkema Inc. and the like.

(2-6) Thermoplastic Polyester Resin and Thermoplastic Polyester Elastomer

The thermoplastic polyester resin is not particularly limited, as long as it is a thermoplastic resin having plurality of ester bonds in the main molecular chain. For example, a product obtained by a reaction between dicarboxylic acid and diol is preferable. Examples of the thermoplastic polyester elastomer include, for example, a block copolymer having a hard segment consisting of a polyester component and a soft segment. Examples of the polyester component constituting the hard segment include, for example, an aromatic polyester. Examples of the soft segment component include an aliphatic polyether, an aliphatic polyester and the like.

Specific examples of the polyester elastomer include "Hytrel 3548", "Hytrel 4047" manufactured by Toray-DuPont Co., Ltd; "Primalloy A1606", "Primalloy B1600", "Primalloy B1700" manufactured by Mitsubishi Chemical Corporation; and the like.

(2-7) Thermoplastic (Meth)Acrylic-Based Elastomer

Examples of the thermoplastic (meth)acrylic-based elastomer include a thermoplastic elastomer obtained by copolymerizing ethylene and (meth)acrylic acid ester. Specific examples of the thermoplastic (meth)acrylic-based elastomer include, for example, "Kurarite (a block copolymer of methyl methacrylate and butyl acrylate)" manufactured by Kuraray Co., Ltd.

The thermoplastic resin composition preferably contains, as the resin component, at least one kind selected from the group consisting of the ionomer resin, the thermoplastic olefin copolymer, the thermoplastic styrene-based elastomer, the thermoplastic polyester elastomer, the thermoplastic polyurethane elastomer, the thermoplastic polyamide elastomer, and the thermoplastic acrylic-based elastomer. This is because a constituent member having a desired hardness can be formed easily.

In the present invention, when the ionomer resin or the thermoplastic olefin copolymer are used as the resin component contained in the thermoplastic resin composition, the thermoplastic resin composition may further contain (B) a basic metal salt of a fatty acid which will be explained below. By containing (B) the basic metal salt of the fatty acid, the degree of neutralization of the ionomer resin and the thermoplastic olefin copolymer can be increased. By increasing the degree of neutralization, the resilience of the resultant constituent member becomes higher.

(B) The basic metal salt of the fatty acid is obtained by a well-known producing method where a fatty acid is allowed to react with a metal oxide or metal hydroxide. The conventional metal salt of the fatty acid is obtained by a reaction of the fatty acid with the metal oxide or metal hydroxide in an amount of the reaction equivalent, whereas (B) the basic metal salt of the fatty acid is obtained by adding the metal oxide or metal hydroxide in an excessive amount which is larger than the reaction equivalent to the fatty acid, and the resultant product has a different metal content, melting point or the like from the conventional metal salt of the fatty acid.

As (B) the basic metal salt of the fatty acid, a basic metal salt of a fatty acid represented by the following general formula (1) is preferred.



In the formula (1),  $m$  represents the number of moles of metal oxides or metal hydroxides in the basic metal salt of the fatty acid. The  $m$  preferably ranges from 0.1 to 2.0, and more preferably from 0.2 to 1.5. If  $m$  is less than 0.1, the resilience of the obtained resin composition may be lowered, while if  $m$  exceeds 2.0, the melting point of the basic metal salt of the fatty acid becomes so high that the basic metal salt of the fatty acid is hardly dispersed in the resin component.  $M^1$  and  $M^2$  are preferably the group II or the group XII metals of the periodic table, respectively.  $M^1$  and  $M^2$  may be identical or different from each other. Examples of the group II metals include beryllium, magnesium, calcium, strontium and barium. Examples of the group XII metals include zinc, cadmium and mercury. Preferred is, for example, magnesium, calcium, barium or zinc, and more preferred is magnesium, as  $M^1$  and  $M^2$  metals.

In the formula (1),  $RCOO$  means the residue of the saturated fatty acid or unsaturated fatty acid. Specific examples of the saturated fatty acid component of (B) the basic metal salt of the fatty acid (IUPAC name) include butanoic acid (C4), pentanoic acid (C5), hexanoic acid (C6), heptanoic acid (C7), octanoic acid (C8), nonanoic acid (C9), decenoic acid (C10), undecenoic acid (C11), dodecenoic acid (C12), tridecanoic acid (C13), tetradecenoic acid (C14), pentadecanoic acid (C15), hexadecanoic acid (C16), heptadecanoic acid (C17), octadecanoic acid (C18), nonadecanoic acid (C19), icosanoic acid (C20), henicosanoic acid (C21), docosanoic acid (C22), tricosanoic acid (C23), tetracosanoic acid (C24), pentacosanoic acid (C25), hexacosanoic acid (C26), heptacosanoic acid (C27), octacosanoic acid (C28), nonacosanoic acid (C29), and triacosanoic acid (C30).

Specific examples of the unsaturated fatty acid component of (B) the basic metal salt of the fatty acid (IUPAC name) include butenoic acid (C4), pentenoic acid (C5), hexenoic acid (C6), heptenoic acid (C7), octenoic acid (C8), nonenoic acid (C9), decenoic acid (C10), undecenoic acid (C11), dodecenoic acid (C12), tridecenoic acid (C13), tetradecenoic acid (C14), pentadecenoic acid (C15), hexadecenoic acid (C16), heptadecenoic acid (C17), octadecenoic acid (C18), nonadecenoic acid (C19), icosenoic acid (C20), henicosenoic acid (C21), docosenoic acid (C22), tricosenoic acid (C23), tetracosenoic acid (C24), pentacosenoic acid (C25), hexacosenoic acid (C26), heptacosenoic acid (C27), octacosenoic acid (C28), nonacosenoic acid (C29), and triacosenoic acid (C30).

Specific examples of the fatty acid component of (B) the basic metal salt of the fatty acid (Common name) are, for example, butyric acid (C4), valeric acid (C5), caproic acid (C6), enanthic acid (C7), caprylic acid (C8), pelargonic acid (C9), capric acid (C10), lauric acid (C12), myristic acid (C14), myristoleic acid (C14), pentadecyclic acid (C15), palmitic acid (C16), palmitoleic acid (C16), margaric acid (C17), stearic acid (C18), elaidic acid (C18), vaccenic acid (C18), oleic acid (C18), linoleic acid (C18), linolenic acid (C18), 12-hydroxy stearic acid (C18), arachidic acid (C20), gadoleic acid (C20), arachidonic acid (C20), eicosenoic acid (C20), behenic acid (C22), erucic acid (C22), lignoceric acid (C24), nervonic acid (C24), cerotic acid (C26), montanic acid (C28), and melissic acid (C30).

(B) The basic metal salt of the fatty acid is preferably a basic metal salt of an unsaturated fatty acid. The unsaturated fatty acid component preferably includes at least one selected from the group consisting of oleic acid (C18), erucic acid (C22), linoleic acid (C18), linolenic acid (C18), arachidonic acid (C20), eicosapentaenoic acid (C20), docosahexaenoic acid (C22), stearidonic acid (C18), nervonic acid (C24), vaccenic acid (C18), gadoleic acid (C20), elaidic acid (C18), eicosenoic acid (C20), eicosadienoic acid (C20), docosadienoic acid (C22), pinolenic acid (C18), eleostearic acid (C18), mead acid (C20), adrenic acid (C22), clupanodonic acid (C22), nisinic acid (C24), and tetracosapentaenoic acid (C24).

(B) The basic metal salt of the fatty acid is preferably a basic metal salt of a fatty acid having 8 to 30 carbon atoms, and more preferably a basic metal salt of a fatty acid having 12 to 24 carbon atoms. Specific examples of (B) the basic metal salt of the fatty acid include basic magnesium laurate, basic calcium laurate, basic zinc laurate, basic magnesium myristate, basic calcium myristate, basic zinc myristate, basic magnesium palmitate, basic calcium palmitate, basic zinc palmitate, basic magnesium oleate, basic calcium oleate, basic zinc oleate, basic magnesium stearate, basic calcium stearate, basic zinc stearate, basic magnesium 12-hydroxystearate, basic calcium 12-hydroxystearate, basic zinc 12-hydroxystearate, basic magnesium behenate, basic calcium behenate, and basic zinc behenate. (B) The basic metal salt of the fatty acid preferably includes a basic magnesium salt of a fatty acid, and more preferably basic magnesium stearate, basic magnesium behenate, basic magnesium laurate, and basic magnesium oleate. (B) The basic metal salt of the fatty acid may be used alone or as a mixture of at least two of them.

There is no particular limitation on the melting point of (B) the basic metal salt of the fatty acid, but if the metal is magnesium, the melting point is preferably 100°C. or more, and is preferably 300°C. or less, more preferably 290°C. or less, even more preferably 280°C. or less. If the melting

point falls within the above range, the dispersibility to the resin component becomes better.

(B) The basic metal salt of the fatty acid preferably contains the metal component in an amount of 1 mole % or more, more preferably 1.1 mole % or more, and preferably contains the metal component in an amount of 2 mole % or less, more preferably 1.9 mole % or less. If the content of the metal component falls within the above range, the resilience of the obtained golf ball's constituent member is further increased. The content of the metal component of (B) the basic metal salt of the fatty acid is a value calculated by dividing the metal amount (g) contained per 1 mole of the metal salt by the atomic weight of the metal, and is expressed in mole %.

The content of (B) the basic metal salt of the fatty acid in the thermoplastic resin composition used in the present invention is preferably 5 parts by mass or more, more preferably 8 parts by mass or more, even more preferably 10 parts by mass or more, and is preferably 100 parts by mass or less, more preferably 90 parts by mass or less, with respect to 100 parts by mass of (A) the resin component. If the content of (B) the basic metal salt of the fatty acid is 5 parts by mass or more, the resilience of the golf ball's constituent member is increased, while if the content is 100 parts by mass or less, it is possible to suppress the lowering of the durability of the golf ball's constituent member due to the increase in the low-molecular weight component.

Examples of the resin component constituting the center or the envelope layers preferably include the ionomer resin, the thermoplastic olefin copolymer, the thermoplastic styrene-based elastomer and the mixture thereof. As the resin component, a resin component containing the thermoplastic styrene-based elastomer is preferable. Examples of the thermoplastic styrene-based elastomer preferably include the alloy of one kind or two or more kinds selected from the group consisting of SBS, SIS, SIBS, SEBS, SEPS, SEEPS and the hydrogenated product thereof with the polyolefin. The content of the thermoplastic styrene-based elastomer in the resin component constituting the center is preferably 5 mass % or more, more preferably 10 mass % or more, and is preferably 100 mass % or less, more preferably 80 mass % or less.

Examples of the preferable embodiment of the resin component constituting the center or the envelope layers include the following embodiments.

(1) An embodiment containing the ionomer resin and the thermoplastic styrene-based elastomer as the resin component. In a more preferable embodiment, the ternary ionomer resin and the alloy of one kind or two or more kinds selected from the group consisting of SBS, SIS, SIBS, SEBS, SEPS, SEEPS and the hydrogenated product thereof with the polyolefin are contained.

(2) An embodiment containing the ionomer resin and the thermoplastic styrene-based elastomer, and further containing the basic metal salt of the fatty acid for increasing the degree of neutralization of the ionomer resin. In a more preferable embodiment, the ternary ionomer resin, the alloy of one kind or two or more kinds selected from the group consisting of SBS, SIS, SIBS, SEBS, SEPS, SEEPS and the hydrogenated product thereof with the polyolefin, and further the basic metal salt of the fatty acid for increasing the degree of neutralization of the ionomer resin are contained.

(3) An embodiment containing the thermoplastic olefin copolymer and the thermoplastic styrene-based elastomer, and further containing the basic metal salt of the fatty acid for increasing the degree of neutralization of the thermoplastic olefin copolymer. Examples of the thermoplastic

olefin copolymer preferably include the binary copolymer composed of the olefin and the  $\alpha,\beta$ -unsaturated carboxylic acid having 3 to 8 carbon atoms and/or the ternary copolymer composed of the olefin, the  $\alpha,\beta$ -unsaturated carboxylic acid having 3 to 8 carbon atoms and the  $\alpha,\beta$ -unsaturated carboxylic acid ester. Examples of the thermoplastic styrene-based elastomer preferably include the alloy of one kind or two or more kinds selected from the group consisting of SBS, SIS, SIBS, SEBS, SEPS, SEEPS and the hydrogenated product thereof with the polyolefin.

The resin component constituting the second envelope layer preferably contains an ionomer resin and a thermoplastic styrene-based elastomer. A total amount of these resin components is preferably 50 mass % or more, more preferably 70 mass % or more, even more preferably 90 mass % or more. In this case, a mass ratio of the ionomer resin to the thermoplastic styrene-based elastomer (ionomer resin/thermoplastic styrene-based elastomer) is preferably 0.1 or more, more preferably 0.2 or more, even more preferably 0.3 or more, and is preferably 3.0 or less, more preferably 1.7 or less, even more preferably 1.2 or less.

The resin component constituting the outermost envelope layer preferably the ionomer resin. The content percentage of the ionomer resin is preferably 50 mass % or more, more preferably 70 mass % or more, even more preferably 90 mass % or more.

The resin component constituting the cover preferably contains an ionomer resin, a thermoplastic polyurethane resin (including a thermoplastic polyurethane elastomer), or a mixture thereof. If the resin component constituting the cover contains the ionomer resin, the golf ball showing excellent durability and travelling a long distance can be obtained. If the resin component constituting the cover contains the thermoplastic polyurethane resin (including a thermoplastic polyurethane elastomer), the golf ball showing excellent shot feeling and controllability can be obtained.

The resin component constituting the cover preferably contains a thermoplastic polyurethane resin. The content percentage of the thermoplastic polyurethane resin is preferably 50 mass % or more, more preferably 70 mass % or more, even more preferably 90 mass % or more.

The thermoplastic resin composition used in the present invention may further contain (C) an additive. Examples of (C) the additive include a pigment component such as a white pigment (for example, titanium oxide), a blue pigment or the like; a weight adjusting agent; a dispersant; an antioxidant; an ultraviolet absorber; a light stabilizer; a fluorescent material; a fluorescent brightener; or the like. Examples of the weight adjusting agent include inorganic fillers such as zinc oxide, barium sulfate, calcium carbonate, magnesium oxide, tungsten powder, molybdenum powder, and the like.

The content of the white pigment (for example, titanium oxide), with respect to 100 parts by mass of (A) the resin component, is preferably 0.5 part by mass or more, more preferably 1 part by mass or more, and is preferably 10 parts by mass or less, more preferably 8 parts by mass or less. If the content of the white pigment is 0.5 part by mass or more, it is possible to impart the opacity to the golf ball's constituent member. If the content of the white pigment is more than 10 parts by mass, the durability of the obtained golf ball's constituent member may deteriorate.

The thermoplastic resin composition used in the present invention can be obtained, for example, by dry blending (A) the resin component and (C) the additive. (B) The basic metal salt of the fatty acid is dry blended where necessary.

Further, the dry blended mixture may be extruded into a pellet form. The dry blending is preferably carried out by using for example, a mixer capable of blending raw materials in a pellet form, more preferably carried out by using a tumbler type mixer. Extruding can be carried out by using a publicly known extruder such as a single-screw extruder, a twin-screw extruder, and a twin-single extruder.

#### Rubber Composition

Next, the rubber composition which can be used in the present invention will be explained. Examples of the rubber composition include a composition containing a base rubber, a crosslinking initiator, a co-crosslinking agent, and a filler.

As the base rubber, a natural rubber and/or a synthetic rubber may be used. Examples of the base rubber include a polybutadiene rubber, a natural rubber, a polyisoprene rubber, a styrene polybutadiene rubber, and an ethylene-propylene-diene rubber (EPDM). These rubbers can be used solely or as a combination of two or more kinds. Among them, particularly preferred is a high cis-polybutadiene having cis-1,4-bond which is beneficial to resilience in a content of 40 mass % or more, more preferably 80 mass % or more, even more preferably 90 mass % or more.

The high cis-polybutadiene preferably has 1,2-vinyl bond in a content of 2 mass or less, more preferably 1.7 mass % or less, and even more preferably 1.5 mass % or less. If the content of 1,2-vinyl bond is excessively high, the resilience may be lowered.

The high cis-polybutadiene preferably includes a product synthesized by using a rare-earth element catalyst. When a neodymium catalyst employing a neodymium compound which is a lanthanum series rare-earth element compound, is used, a polybutadiene rubber having a high content of cis-1,4 bond and a low content of 1,2-vinyl bond can be obtained with excellent polymerization activity, thus such a polybutadiene rubber is particularly preferred.

The high cis-polybutadiene preferably has a Mooney viscosity (ML<sub>1+4</sub> (100° C.)) of 30 or more, more preferably 32 or more, even more preferably 35 or more, and preferably has a Mooney viscosity (ML<sub>1+4</sub> (100° C.)) of 140 or less, more preferably 120 or less, even more preferably 100 or less, most preferably 80 or less. It is noted that the Mooney viscosity (ML<sub>1+4</sub> (100° C.)) in the present invention is a value measured according to JIS K6300 using an L rotor under the conditions of: a preheating time of 1 minute; a rotor rotation time of 4 minutes; and a temperature of 100° C.

The high cis-polybutadiene preferably has a molecular weight distribution Mw/Mn (Mw: weight average molecular weight, Mn: number average molecular weight) of 2.0 or more, more preferably 2.2 or more, even more preferably 2.4 or more, most preferably 2.6 or more, and preferably has a molecular weight distribution Mw/Mn of 6.0 or less, more preferably 5.0 or less, even more preferably 4.0 or less, most preferably 3.4 or less. If the molecular weight distribution (Mw/Mn) of the high cis-polybutadiene is excessively low, the processability may deteriorate. If the molecular weight distribution (Mw/Mn) of the high cis-polybutadiene is excessively high, the resilience may be lowered. It is noted that the molecular weight distribution is measured by gel permeation chromatography ("HLC-8120GPC" manufactured by Tosoh Corporation) using a differential refractometer as a detector under the conditions of column: GMH-HXL (manufactured by Tosoh Corporation), column temperature: 40° C., and mobile phase: tetrahydrofuran, and calculated by converting based on polystyrene standard.

The crosslinking initiator is blended to crosslink the base rubber component. As the crosslinking initiator, an organic

peroxide is preferably used. Specific examples of the organic peroxide are dicumyl peroxide, 1,1-bis(t-butylperoxy)-3,3,5-trimethylcyclohexane, 2,5-dimethyl-2,5-di(t-butylperoxy)hexane, and di-t-butyl peroxide. Among them, dicumyl peroxide is preferably used. The blending amount of the crosslinking initiator is preferably 0.3 part by mass or more, more preferably 0.4 part by mass or more, and is preferably 5 parts by mass or less, more preferably 3 parts by mass or less, with respect to 100 parts by mass of the base rubber. If the amount is less than 0.3 part by mass, the resultant envelope layer becomes so soft that the resilience tends to be lowered, and if the amount is more than 5 parts by mass, the amount of the co-crosslinking agent must be decreased to obtain an appropriate hardness, which tends to cause the insufficient resilience.

The co-crosslinking agent is considered to have an action of crosslinking a rubber molecule by graft polymerization to a base rubber molecular chain. As the co-crosslinking agent, for example, an α,β-unsaturated carboxylic acid having 3 to 8 carbon atoms or a metal salt thereof can be used, examples thereof preferably include acrylic acid, methacrylic acid and a metal salt thereof. Examples of the metal constituting the metal salt include, for example, zinc, magnesium, calcium, aluminum and sodium, among them, zinc is preferably used because it provides high resilience.

The amount of the co-crosslinking agent to be used is preferably 10 parts by mass or more, more preferably 15 parts by mass or more, even more preferably 20 parts by mass or more, and is preferably 55 parts by mass or less, more preferably 50 parts by mass or less, even more preferably 48 parts by mass or less, with respect to 100 parts by mass of the base rubber. If the amount of the co-crosslinking agent to be used is less than 10 parts by mass, the amount of the crosslinking initiator must be increased to obtain an appropriate hardness, which tends to lower the resilience. On the other hand, if the amount of the co-crosslinking agent to be used is more than 55 parts by mass, the resultant envelope layer becomes so hard that the shot feeling may be lowered.

The filler contained in the rubber composition is mainly blended as a weight adjusting agent in order to adjust the weight of the golf ball obtained as a final product, and may be blended where necessary. Examples of the filler include an inorganic filler such as zinc oxide, barium sulfate, calcium carbonate, magnesium oxide, tungsten powder, and molybdenum powder. The blending amount of the filler is preferably 0.5 part by mass or more, more preferably 1 part by mass or more, and is preferably 30 parts by mass or less, more preferably 20 parts by mass or less, with respect to 100 parts by mass of the base rubber. If the blending amount of the filler is less than 0.5 part by mass, it becomes difficult to adjust the weight, while if it is more than 30 parts by mass, the weight fraction of the rubber component becomes small and the resilience tends to be lowered.

An organic sulfur compound, an antioxidant, a peptizing agent or the like may be blended appropriately in the rubber composition, in addition to the base rubber, the crosslinking initiator, the co-crosslinking agent and the filler.

Examples of the organic sulfur compound include thiophenols, thionaphthols, polysulfides, thiocarboxylic acids, dithiocarboxylic acids, sulfenamides, thiurams, dithiocarbamates, thiazoles, and the like. Among them, diphenyl disulfides may be preferably used as the organic sulfur compound. Examples of the diphenyl disulfides include diphenyl disulfide; a mono-substituted diphenyl disulfide such as bis(4-chlorophenyl)disulfide, bis(3-chlorophenyl)disulfide, bis(4-bromophenyl)disulfide, bis(3-bromophenyl)

disulfide, bis(4-fluorophenyl)disulfide, bis(4-iodophenyl)disulfide, bis(4-cyanophenyl)disulfide; a di-substituted diphenyl disulfide such as bis(2,5-dichlorophenyl)disulfide, bis(3,5-dichlorophenyl)disulfide, bis(2,6-dichlorophenyl)disulfide, bis(2,5-dibromophenyl)disulfide, bis(3,5-dibromophenyl)disulfide, bis(2-chloro-5-bromophenyl)disulfide, bis(2-cyano-5-bromophenyl)disulfide; a tri-substituted diphenyl disulfide such as bis(2,4,5-trichlorophenyl)disulfide, bis(2,4,6-trichlorophenyl)disulfide, bis(2-cyano-4-chloro-6-bromophenyl)disulfide; a tetra-substituted diphenyl disulfide such as bis(2,3,5,6-tetra chlorophenyl)disulfide; a penta-substituted diphenyl disulfide such as bis(2,3,4,5,6-pentachlorophenyl)disulfide, bis(2,3,4,5,6-pentabromophenyl)disulfide. These diphenyl disulfides can enhance resilience by having some influence on the state of vulcanization of vulcanized rubber. Among them, diphenyl disulfide or bis(pentabromophenyl) disulfide is preferably used since the golf ball having particularly high resilience can be obtained. The blending amount of the organic sulfur compound is preferably 0.1 part by mass or more, more preferably 0.3 part by mass or more, and is preferably 5.0 parts by mass or less, more preferably 3.0 parts by mass or less, with respect to 100 parts by mass of the base rubber.

The blending amount of the antioxidant is preferably 0.1 part by mass or more and 1 part by mass or less with respect to 100 parts by mass of the base rubber. Further, the blending amount of the peptizing agent is preferably 0.1 part by mass or more and 5 parts by mass or less with respect to 100 parts by mass of the base rubber.

The raw materials are mixed and kneaded, and the resultant rubber composition is molded into the envelope layer in a mold. Examples of the method for molding the rubber composition into the envelope layer include, without particular limitation, a method comprising the steps of: molding the rubber composition into a half shell having a hemispherical shape beforehand, covering the golf ball body with two half shells, and compression molding at 130° C. to 170° C. for 5 minutes to 30 minutes; and a method of injection molding the rubber composition.

Examples of the structure of the multi-piece golf ball according to the present invention include: a four-piece golf ball comprising a spherical center, two envelope layers covering the spherical center, and a cover covering the envelope layers; a five-piece golf ball comprising a spherical center, three envelope layers covering the spherical center, and a cover covering the envelope layers; a six-piece golf ball comprising a spherical center, four envelope layers covering the spherical center, and a cover covering the envelope layers; and a seven-piece golf ball comprising a spherical center, five envelope layers covering the spherical center, and a cover covering the envelope layers; and the like.

Examples of the constituent material combination of the golf ball include: an embodiment in which the spherical center and the second envelope layer (E2) are formed from the thermoplastic resin composition; an embodiment in which the spherical center and the second envelope layer (E2) are formed from the rubber composition; an embodiment in which the spherical center is formed from the thermoplastic resin composition, and the second envelope layer (E2) is formed from the rubber composition; an embodiment in which the spherical center is formed from the rubber composition, and the second envelope layer (E2) is formed from the thermoplastic resin composition; and the like. It is preferable that the first envelope layer (E1) and the outermost envelope layer (En) are formed from the thermoplastic resin composition.

FIG. 3 is a partially cutaway view of a golf ball 1 of one embodiment according to the present invention. The golf ball 1 comprises a spherical center 2, a first envelope layer 3 disposed on the outer side of the spherical center 2, a second envelope layer 4 disposed on the outer side of the first envelope 3, a third envelope layer 5 disposed on the outer side of the second envelope 4, a fourth envelope layer 6 disposed on the outer side of the third envelope 5, a fifth envelope layer 7 disposed on the outer side of the fourth envelope 6, and a cover 8 disposed on the outer side of the fifth envelope layer 7. A plurality of dimples 81 are formed on the surface of the cover 8. Other portions than dimples 81 on the surface of the cover 8 are land 82.

(3) Method for Producing Multi-Piece Golf Ball Center

The thermoplastic resin composition or the rubber composition can be used as the center constituent material. In the case that the center is formed from the thermoplastic resin composition, the center can be obtained, for example, by injection molding the thermoplastic resin composition. Specifically, it is preferred that the thermoplastic resin composition heated and melted at a temperature of 160° C. to 260° C. is charged into a mold held under a pressure of 1 MPa to 100 MPa for 1 second to 100 seconds, and after cooling for 30 second to 300 seconds, the mold is opened.

In the case that the center is formed from the rubber composition, the center can be obtained by molding the kneaded rubber composition in a mold. The temperature for molding the spherical center is preferably 120° C. to 170° C. The molding pressure is preferably 2.9 MPa to 11.8 MPa, and the molding time is preferably 10 minutes to 60 minutes. Envelope Layer

The thermoplastic resin composition or the rubber composition can be used as the envelope layer constituent material. In the case that the envelope layer is formed from the thermoplastic resin composition, the envelope layer can be obtained, for example, by a method of molding the thermoplastic resin composition into a half shell having a hemispherical shape beforehand, covering the spherical body with two half shells, and compression molding at 130° C. to 170° C. for 1 minute to 5 minutes, or by a method of directly injection molding the thermoplastic resin composition onto the spherical body to cover the center therein.

When injection molding the thermoplastic resin composition onto the spherical body to mold the envelope layer, it is preferred to use upper and lower molds having a hemispherical cavity and a hold pin. Injection molding of the envelope layer can be carried out by protruding the hold pin to hold the spherical body, charging the heated and melted thermoplastic resin composition and then cooling to obtain the envelope layer.

When molding the envelope layer by compression molding method, the half shell can be molded by either compression molding method or injection molding method, but compression molding method is preferred. Compression molding the thermoplastic resin composition into the half shell can be carried out, for example, under a pressure of 1 MPa or more and 20 MPa or less at a molding temperature of -20° C. or more and 70° C. or less relative to the flow beginning temperature of the thermoplastic resin composition. By carrying out the molding under the above conditions, the half shell with a uniform thickness can be formed. Examples of the method for molding the envelope layer with half shells include a method of covering the spherical body with two half shells and then performing compression molding. Compression molding the half shells into the envelope layer can be carried out, for example, under a

21

molding pressure of 0.5 MPa or more and 25 MPa or less at a molding temperature of  $-20^{\circ}\text{C}$ . or more and  $70^{\circ}\text{C}$ . or less relative to the flow beginning temperature of the thermoplastic resin composition. By carrying out the molding under the above conditions, the envelope layer with a uniform thickness can be formed.

The molding temperature means the highest temperature where the temperature at the surface of the concave portion of the lower mold reaches from closing the mold to opening the mold. Further, the flow beginning temperature of the thermoplastic resin composition can be measured in a pellet form under the following conditions by using "Flow Tester CFT-500" manufactured by Shimadzu Corporation. Measuring conditions: Plunger Area: 1 cm<sup>2</sup>, Die length: 1 mm, Die diameter: 1 mm, Load: 588.399 N, Start temperature: 30° C., and Temperature increase rate: 3° C./min.

When the envelope layer is formed from the rubber composition, the envelope layer can be obtained, for example, by a method of molding the rubber composition into a half shell having a hemispherical shape beforehand, covering the spherical body with two half shells, and compression molding at 130° C. to 170° C. for 5 minutes to 30 minutes. The envelope layer may also be formed by injection molding the rubber composition.

Cover

The thermoplastic resin composition can be used as the cover constituent material. As the method of molding the thermoplastic resin composition into the cover, the above-described method of molding the thermoplastic resin composition into the envelope layer can be adopted. It is preferred to use upper and lower molds having a hemispherical cavity and pimples wherein a part of the pimple also serves as a retractable hold pin.

The concave portions called "dimple" are usually formed on the surface of the cover. The total number of dimples formed on the cover is preferably 200 or more and 500 or less. If the total number of dimples is less than 200, the dimple effect is hardly obtained. On the other hand, if the total number of dimples exceeds 500, the dimple effect is hardly obtained because the size of the respective dimple is small. The shape (shape in a plan view) of dimples includes, without limitation, a circle; a polygonal shape such as a roughly triangular shape, a roughly quadrangular shape, a roughly pentagonal shape, a roughly hexagonal shape; or other irregular shape. The shape of dimples is employed solely or in combination of at least two of them.

After the cover is molded, the obtained golf ball body is ejected from the mold, and is preferably subjected to surface treatments such as deburring, cleaning and sandblast where necessary. If desired, a paint film or a mark may be formed. The paint film preferably has a thickness of, but not limited to, 5  $\mu\text{m}$  or larger, and more preferably 7  $\mu\text{m}$  or larger, and preferably has a thickness of 50  $\mu\text{m}$  or smaller, more preferably 40  $\mu\text{m}$  or smaller, even more preferably 30  $\mu\text{m}$  or smaller. If the thickness of the paint film is smaller than 5  $\mu\text{m}$ , the paint film is easy to wear off due to continued use of the golf ball, and if the thickness of the paint film is larger

22

than 50  $\mu\text{m}$ , the dimple effect is reduced, resulting in lowering flying performance of the golf ball.

## Examples

Hereinafter, the present invention will be described in detail by way of example. The present invention is not limited to examples described below. Various changes and modifications can be made without departing from the spirit and scope of the present invention.

## 10 [Evaluation Method]

### Material Hardness (Shore D Hardness)

In case of the thermoplastic resin composition, sheets with a thickness of about 2 mm were produced by injection molding, and in case of the rubber composition, sheets with a thickness of about 2 mm were produced by compressing at 170° C. for 25 minutes. These sheets were stored at 23° C. for two weeks. Three or more of these sheets were stacked on one another so as not to be affected by the measuring substrate on which the sheets were placed, and the hardness of the stack was measured with a type P1 auto loading durometer manufactured by Kobunshi Keiki Co., Ltd., provided with a Shore D type spring hardness tester prescribed in ASTM-D2240.

### Compression Deformation Amount (mm)

The compression deformation amount of the golf ball along the compression direction (shrinking amount of the golf ball along the compression direction), when applying a load from 98 N as an initial load to 1275 N as a final load to the golf ball, was measured.

### Spin Rate (Rpm) on Driver Shots

A metal-headed W #1 driver (XXIO S, loft: 11°, manufactured by Dunlop Sports Limited) was installed on a swing robot M/C manufactured by Golf Laboratories, Inc. The golf ball was hit at a head speed of 50 m/sec, and the spin rate right after hitting the golf ball was measured. This measurement was conducted twelve times for each golf ball, and the average value thereof was adopted as the measurement value for the golf ball. A sequence of photographs of the hit golf ball were taken for measuring the spin rate right after hitting the golf ball.

### Spin Rate on Approach Shots

40 A sand wedge (CG15 forged wedge ( $58^\circ$ ), manufactured by Cleveland Golf) was installed on a swing machine manufactured by True Temper Sports, Inc. The golf ball was hit at a head speed of 10 m/sec, and the spin rate (rpm) was measured by taking a sequence of photographs of the hit golf ball. This measurement was conducted ten times for each golf ball, and the average value thereof was adopted as the spin rate.

## [Preparation of Thermoplastic Resin Composition]

As shown in Table 1, the blending materials were dry blended, followed by mixing with a twin-screw kneading extruder to extrude the blended material in a strand form into the cool water. The extruded strand was cut with a pelletizer to prepare the thermoplastic resin composition in a pellet form. Extrusion was performed in the following conditions: screw diameter: 45 mm, screw revolutions: 200 rpm; and screw L/D=35. The blending materials were heated to a temperature in a range from 160° C. to 230° C. at the die position of the extruder.

TABLE 1

TABLE 1-continued

|                         | Thermoplastic resin composition No. |     |     |     |     |     |     |     |     |    |     |
|-------------------------|-------------------------------------|-----|-----|-----|-----|-----|-----|-----|-----|----|-----|
|                         | a                                   | b   | c   | d   | e   | f   | g   | h   | i   | k  | l   |
| Himilan AM7329          | —                                   | —   | —   | —   | —   | —   | —   | —   | —   | 50 | —   |
| HPF2000                 | 100                                 | —   | —   | —   | 75  | 60  | 50  | 25  | —   | —  | —   |
| HPF1000                 | —                                   | 100 | —   | —   | —   | —   | —   | —   | —   | —  | —   |
| Rabalon T3221C          | —                                   | —   | 50  | 60  | 25  | 40  | 50  | 75  | 100 | —  | —   |
| Elastollan XNY84A       | —                                   | —   | —   | —   | —   | —   | —   | —   | —   | —  | 100 |
| Basic Mg oleate         | —                                   | —   | 15  | 28  | —   | —   | —   | —   | —   | —  | —   |
| Titanium oxide          | —                                   | —   | —   | —   | —   | —   | —   | —   | —   | 4  | 4   |
| Shore D hardness        | 45                                  | 54  | 27  | 23  | 35  | 29  | 25  | 15  | 5   | 65 | 32  |
| Ionomer resin/          | —                                   | —   | 1.0 | 0.7 | 3.0 | 1.5 | 1.0 | 0.3 | —   | —  | —   |
| Styrene-based elastomer | —                                   | —   | —   | —   | —   | —   | —   | —   | —   | —  | —   |

15

The materials used in Table 1 are follows.

Himilan AM7327: zinc ion-neutralized ethylene-methacrylic acid-butyl acrylate ternary copolymer ionomer resin (melt flow rate (190° C., 2.16 kgf): 0.7 g/10 min, bending stiffness: 35 MPa) manufactured by Mitsui-Du Pont Polymers Co., Ltd.

Titanium oxide: A220 manufactured by Ishihara Sangyo Co., Ltd.

[Preparation of Rubber Composition]

20 The materials shown in Table 2 were mixed and kneaded to prepare the rubber composition.

TABLE 2

|                                |                                    | Rubber composition No. |                       |                       |                       |                       |
|--------------------------------|------------------------------------|------------------------|-----------------------|-----------------------|-----------------------|-----------------------|
|                                |                                    | A                      | B                     | C                     | D                     | E                     |
| Formulation<br>(parts by mass) | Polybutadiene rubber               | 100                    | 100                   | 100                   | 100                   | 100                   |
|                                | Zinc acrylate                      | 18                     | 37                    | 10                    | 5                     | 20                    |
|                                | Zinc oxide                         | 5                      | 5                     | 5                     | 5                     | 5                     |
|                                | Diphenyl disulfide                 | 0.5                    | —                     | 0.5                   | 0.5                   | 0.5                   |
|                                | Bis(pentabromophenyl)<br>disulfide | —                      | 0.3                   | —                     | —                     | —                     |
|                                | Dicumyl peroxide                   | 0.7                    | 0.9                   | 0.7                   | 0.7                   | 0.7                   |
|                                | Barium sulfate                     | Appropriate<br>amount  | Appropriate<br>amount | Appropriate<br>amount | Appropriate<br>amount | Appropriate<br>amount |
|                                | Shore D hardness                   | 34                     | 51                    | 27                    | 19                    | 45                    |

Nucrel AN4319: ethylene-methacrylic acid-butyl acrylate copolymer (melt flow rate (190° C., 2.16 kgf): 55 g/10 min, bending stiffness: 21 MPa) manufactured by Mitsui-Du Pont Polymers Co., Ltd.

The materials used in Table 2 are follows.  
40 Polybutadiene rubber: "BR-730 (high-cis polybutadiene, cis-1,4 bond content=96 mass %, 1,2-vinyl bond content=1.3 mass %, Moony viscosity (ML<sub>1+4</sub> (100° C.)=55, molecular weight distribution (Mw/Mn)=3)" manufactured by JSR Corporation Zinc acrylate: "ZNDA-90S" manufactured by Nihon Jyoryu Kogyo Co., Ltd.

Himilan 1605: sodium ion-neutralized ethylene-methacrylic acid copolymer ionomer resin (melt flow rate (190° C., 2.16 kgf): 2.8 g/10 min, bending stiffness: 320 MPa) manufactured by Mitsui-Du Pont Polymers Co., Ltd.

Zinc oxide: "Ginrei (registered trademark) R" manufactured by Toho Zinc Co., Ltd.

Himilan AM7329: zinc ion-neutralized ethylene-methacrylic acid copolymer ionomer resin (melt flow rate (190° C., 2.16 kgf): 5 g/10 min, bending stiffness: 221 MPa) manufactured by Mitsui-Du Pont Polymers Co., Ltd.

Diphenyl disulfide: manufactured by Sumitomo Seika Chemicals Co., Ltd.

HPF2000: magnesium ion-neutralized ternary copolymer ionomer resin (melt flow rate (190° C., 2.16 kgf): 1.0 g/10 min, bending stiffness: 64 MPa) manufactured by E.I. du Pont de Nemours and Company

Dicumyl peroxide: "Percumyl (registered trademark) D" manufactured by NOF Corporation

HPF1000: magnesium ion-neutralized ternary copolymer ionomer resin (melt flow rate (190° C., 2.16 kgf): 0.7 g/10 min, bending stiffness: 190 MPa) manufactured by E.I. du Pont de Nemours and Company

Barium sulfate: "Barium Sulfate BD" manufactured by Sakai Chemical Industry Co., Ltd.

Rabalon T3221C: thermoplastic styrene elastomer (alloy of one kind or two or more kinds selected from the group consisting of SBS, SIS, SIBS, SEBS, SEPS, SEEPS and a hydrogenated product thereof with a polyolefin) manufactured by Mitsubishi Chemical Corporation

[Production of Golf Ball]

Elastollan XNY84A: thermoplastic polyurethane elastomer manufactured by BASF Japan Ltd.

(i) Spherical Center

Basic Mg oleate: (metal content: 1.7 mole %; in the formula (1), M<sup>1</sup>=M<sup>2</sup>=Mg, R=17 carbon atoms) manufactured by Nitto Kasei Kougyo Co., Ltd.

Center Formed from Thermoplastic Resin Composition

The thermoplastic resin composition in a pellet form was injection molded at 200° C. to produce the spherical center.

Center Formed from Rubber Composition

60 The rubber composition was heat-pressed at 170° C. for 20 minutes in upper and lower molds having a hemispherical cavity to produce the spherical center.

(ii) Envelope Layer

Envelope Layer Formed from Thermoplastic Resin Composition

65 The thermoplastic resin composition in a pellet form was injection molded at 200° C. to mold the envelope layer. It is

noted that each envelope layer was molded one by one. The utilized upper and lower molds have a hemispherical cavity and a retractable hold pin for holding the spherical body. Molding of the envelope layer was carried out by protruding the hold pin to hold the spherical body, charging the thermoplastic resin composition into the molds, cooling and then opening the molds to eject the spherical body.

## Envelope Layer Formed from Rubber Composition

The rubber composition was molded into half shells, and the spherical body was covered with two half shells. The spherical body and the half shells were charged together into the mold consisting of upper and lower molds which have a hemispherical cavity, and then heated at 170° C. for 25 minutes to produce the envelope layer from the rubber composition.

(iii) Cover

The cover was formed by compression molding the obtained thermoplastic resin composition. Thermoplastic resin composition in a pellet form was charged into each concave portion of the lower mold of the mold which is used

for molding the half shell, and compression was performed to form the half shell. Compression molding was conducted at the molding temperature of 160° C., the molding time of 2 minutes, and the molding pressure of 11 MPa. The 5 spherical body on which the envelope layers have been formed was concentrically covered with two half shells, then charged into the mold having a plurality of pimples on one surface of the cavity thereof, and compression molded to form the cover. Compression molding was conducted at the 10 molding temperature of 150° C., the molding time of 3 minutes and the molding pressure of 13 MPa. A plurality of dimples having a reversed shape of the pimple shape were formed on the molded cover.

(iv) Paint

15 The surface of the obtained golf ball body was treated with sandblast, marked, and painted with a clear paint. The paint was dried in an oven at 40° C. to obtain the golf ball. The thickness and material hardness of each layer, and the evaluation results of the golf ball were shown in Tables 3 to 6.

TABLE 3

| Golf ball No.                 |                                     |      |      |      |      |      |      |      |      |
|-------------------------------|-------------------------------------|------|------|------|------|------|------|------|------|
|                               |                                     | 1-1  | 1-2  | 1-3  | 1-4  | 1-5  | 1-6  | 1-7  | 1-8  |
| Center                        | Material No.                        | e    | e    | e    | a    | c    | e    | f    | f    |
|                               | Hardness H0 (Shore D)               | 35   | 35   | 35   | 45   | 27   | 35   | 29   | 29   |
|                               | Diameter (mm)                       | 15   | 15   | 15   | 15   | 15   | 15   | 15   | 20   |
| First envelope layer          | Material No.                        | f    | f    | g    | f    | g    | f    | a    | a    |
|                               | Hardness H1 (Shore D)               | 29   | 29   | 25   | 29   | 25   | 29   | 45   | 45   |
|                               | Thickness (mm)                      | 2.5  | 2.5  | 2.5  | 2.5  | 2.5  | 2.5  | 2.5  | 2.5  |
| Second envelope layer         | Material No.                        | h    | h    | h    | h    | h    | h    | g    | d    |
|                               | Hardness H2 (Shore D)               | 15   | 15   | 15   | 15   | 15   | 15   | 25   | 23   |
|                               | Thickness (mm)                      | 2.5  | 2.5  | 2.5  | 2.5  | 2.5  | 2.5  | 2.5  | 2.5  |
| Third envelope layer          | Material No.                        | a    | a    | a    | a    | a    | a    | a    | a    |
|                               | Hardness H3 (Shore D)               | 45   | 45   | 45   | 45   | 45   | 45   | 45   | 45   |
|                               | Thickness (mm)                      | 2.5  | 5.0  | 2.5  | 2.5  | 2.5  | 5.0  | 5.0  | 2.5  |
| Fourth envelope layer         | Material No.                        | b    | b    | b    | b    | b    | b    | b    | b    |
|                               | Hardness H4 (Shore D)               | 54   | 54   | 54   | 54   | 54   | 54   | 54   | 54   |
|                               | Thickness (mm)                      | 4.9  | 2.4  | 4.9  | 4.9  | 4.9  | 2.4  | 2.4  | 2.4  |
| Fifth envelope layer          | Material No.                        | k    | k    | k    | k    | k    | k    | k    | k    |
|                               | Hardness Hn (Shore D)               | 65   | 65   | 65   | 65   | 65   | 65   | 65   | 65   |
|                               | Thickness (mm)                      | 1.0  | 1.0  | 1.0  | 1.0  | 1.0  | 1.0  | 1.0  | 1.0  |
| Cover                         | Material No.                        | 1    | 1    | 1    | 1    | 1    | 1    | 1    | 1    |
|                               | Hardness Hc (Shore D)               | 32   | 32   | 32   | 32   | 32   | 32   | 32   | 32   |
|                               | Thickness (mm)                      | 0.5  | 0.5  | 0.5  | 0.5  | 0.5  | 0.5  | 0.5  | 0.5  |
| Hardness difference (H0 - H2) |                                     | 20   | 20   | 20   | 30   | 12   | 20   | 4    | 6    |
| Hardness difference (H1 - H2) |                                     | 14   | 14   | 10   | 14   | 10   | 14   | 20   | 22   |
| Hardness difference (Hn - H2) |                                     | 50   | 50   | 50   | 50   | 50   | 50   | 40   | 42   |
| Physical properties           | Compression deformation amount (mm) | 2.72 | 2.80 | 2.73 | 2.70 | 2.75 | 2.82 | 2.80 | 2.83 |
|                               | Driver spin rate Sd (rpm)           | 2371 | 2367 | 2316 | 2445 | 2246 | 2312 | 2582 | 2428 |
|                               | Approach spin rate Sa10 (rpm)       | 3799 | 3749 | 3802 | 3801 | 3801 | 3751 | 3712 | 3512 |
|                               | Sd/Sa10                             | 0.62 | 0.63 | 0.61 | 0.64 | 0.59 | 0.62 | 0.70 | 0.69 |

TABLE 3-continued

|                               | Material No.                        | k    | k    | k    | k    | k    | k    | k    |
|-------------------------------|-------------------------------------|------|------|------|------|------|------|------|
| Fifth envelope                | Hardness Hn (Shore D)               | 65   | 65   | 65   | 65   | 65   | 65   | 65   |
| layer                         | Thickness (mm)                      | 1.0  | 1.0  | 1.0  | 1.0  | 1.0  | 1.0  | 1.0  |
| Cover                         | Material No.                        | l    | l    | l    | l    | l    | l    | l    |
|                               | Hardness Hc (Shore D)               | 32   | 32   | 32   | 32   | 32   | 32   | 32   |
|                               | Thickness (mm)                      | 0.5  | 0.5  | 0.5  | 0.5  | 0.5  | 0.5  | 0.5  |
| Hardness difference (H0 - H2) | 14                                  | 14   | 22   | 10   | 4    | -16  | 0    | -16  |
| Hardness difference (H1 - H2) | 30                                  | 30   | 40   | 30   | 20   | 0    | -20  | -20  |
| Hardness difference (Hn - H2) | 50                                  | 50   | 60   | 50   | 40   | 20   | 20   | 20   |
| Physical properties           | Compression deformation amount (mm) | 2.86 | 2.90 | 2.79 | 2.84 | 2.82 | 2.64 | 2.45 |
|                               | Driver spin rate Sd (rpm)           | 2478 | 2382 | 2389 | 2469 | 2573 | 2755 | 2708 |
|                               | Approach spin rate Sa10 (rpm)       | 3739 | 3465 | 3701 | 3739 | 3523 | 3667 | 3678 |
|                               | Sd/Sa10                             | 0.66 | 0.69 | 0.65 | 0.66 | 0.73 | 0.75 | 0.74 |
|                               |                                     | 0.70 |      |      |      |      |      |      |

TABLE 4

|                               |                                     | Golf ball No. |      |      |      |      |
|-------------------------------|-------------------------------------|---------------|------|------|------|------|
|                               |                                     | 2-1           | 2-2  | 2-3  | 2-4  | 2-5  |
| Center                        | Material No.                        | A             | A    | A    | E    | A    |
|                               | Hardness H0 (Shore D)               | 34            | 34   | 34   | 45   | 34   |
|                               | Diameter (mm)                       | 15            | 15   | 15   | 15   | 15   |
| First envelope                | Material No.                        | f             | f    | g    | g    | f    |
| layer                         | Hardness H1 (Shore D)               | 29            | 29   | 25   | 25   | 29   |
|                               | Thickness (mm)                      | 2.5           | 2.5  | 2.5  | 2.5  | 2.5  |
| Second envelope               | Material No.                        | C             | C    | D    | D    | C    |
| layer                         | Hardness H2 (Shore D)               | 27            | 27   | 19   | 19   | 27   |
|                               | Thickness (mm)                      | 2.5           | 2.5  | 2.5  | 2.5  | 2.5  |
| Third envelope                | Material No.                        | a             | a    | a    | a    | a    |
| layer                         | Hardness H3 (Shore D)               | 45            | 45   | 45   | 45   | 45   |
|                               | Thickness (mm)                      | 2.5           | 5.0  | 2.5  | 5.0  | 5.0  |
| Fourth envelope               | Material No.                        | b             | b    | b    | b    | b    |
| layer                         | Hardness H4 (Shore D)               | 54            | 54   | 54   | 54   | 54   |
|                               | Thickness (mm)                      | 4.9           | 2.4  | 4.9  | 2.4  | 2.4  |
| Fifth envelope                | Material No.                        | k             | k    | k    | k    | k    |
| layer                         | Hardness Hn (Shore D)               | 65            | 65   | 65   | 65   | 65   |
|                               | Thickness (mm)                      | 1.0           | 1.0  | 1.0  | 1.0  | 1.0  |
| Cover                         | Material No.                        | l             | l    | l    | l    | l    |
|                               | Hardness Hc (Shore D)               | 32            | 32   | 32   | 32   | 32   |
|                               | Thickness (mm)                      | 0.5           | 0.5  | 0.5  | 0.5  | 0.5  |
| Hardness difference (H0 - H2) | 7                                   | 7             | 15   | 26   | 7    |      |
| Hardness difference (H1 - H2) | 2                                   | 2             | 6    | 6    | 2    |      |
| Hardness difference (Hn - H2) | 38                                  | 38            | 46   | 46   | 38   |      |
| Physical properties           | Compression deformation amount (mm) | 2.71          | 2.80 | 2.73 | 2.71 | 2.81 |
|                               | Driver spin rate Sd (rpm)           | 2377          | 2373 | 2322 | 2357 | 2318 |
|                               | Approach spin rate Sa10 (rpm)       | 3797          | 3746 | 3799 | 3800 | 3749 |
|                               | Sd/Sa10                             | 0.63          | 0.63 | 0.61 | 0.62 | 0.62 |

|                 |                       | Golf ball No. |     |     |     |      |      |
|-----------------|-----------------------|---------------|-----|-----|-----|------|------|
|                 |                       | 2-6           | 2-7 | 2-8 | 2-9 | 2-10 | 2-11 |
| Center          | Material No.          | A             | A   | A   | A   | A    | A    |
|                 | Hardness H0 (Shore D) | 34            | 34  | 34  | 34  | 34   | 34   |
|                 | Diameter (mm)         | 15            | 15  | 20  | 15  | 15   | 15   |
| First envelope  | Material No.          | a             | a   | a   | a   | g    | g    |
| layer           | Hardness H1 (Shore D) | 45            | 45  | 45  | 45  | 25   | 25   |
|                 | Thickness (mm)        | 2.5           | 2.5 | 5.0 | 2.5 | 2.5  | 2.5  |
| Second envelope | Material No.          | C             | D   | C   | E   | E    | E    |
| layer           | Hardness H2 (Shore D) | 27            | 19  | 27  | 45  | 45   | 45   |
|                 | Thickness (mm)        | 2.5           | 2.5 | 2.5 | 7.5 | 7.5  | 7.5  |
| Third envelope  | Material No.          | a             | a   | —   | —   | —    | —    |
| layer           | Hardness H3 (Shore D) | 45            | 45  | —   | —   | —    | —    |
|                 | Thickness (mm)        | 5.0           | 5.0 | —   | —   | —    | —    |
| Fourth envelope | Material No.          | b             | b   | b   | b   | b    | g    |
| layer           | Hardness H4 (Shore D) | 54            | 54  | 54  | 54  | 54   | 25   |
|                 | Thickness (mm)        | 2.4           | 2.4 | 2.4 | 2.4 | 2.4  | 2.4  |
| Fifth envelope  | Material No.          | k             | k   | k   | k   | k    | k    |
| layer           | Hardness Hn (Shore D) | 65            | 65  | 65  | 65  | 65   | 65   |
|                 | Thickness (mm)        | 1.0           | 1.0 | 1.0 | 1.0 | 1.0  | 1.0  |
| Cover           | Material No.          | l             | l   | l   | l   | l    | l    |
|                 | Hardness Hc (Shore D) | 32            | 32  | 32  | 32  | 32   | 32   |
|                 | Thickness (mm)        | 0.5           | 0.5 | 0.5 | 0.5 | 0.5  | 0.5  |

TABLE 4-continued

|                               |                                     |      |      |      |      |      |
|-------------------------------|-------------------------------------|------|------|------|------|------|
| Hardness difference (Ho - H2) | 7                                   | 15   | 7    | -11  | -11  | -11  |
| Hardness difference (H1 - H2) | 18                                  | 26   | 18   | 0    | -20  | -20  |
| Hardness difference (Hn - H2) | 38                                  | 46   | 38   | 20   | 20   | 20   |
| Physical properties           | Compression deformation amount (mm) | 2.76 | 2.79 | 3.04 | 2.76 | 2.78 |
| Driver spin rate Sd (rpm)     | 2545                                | 2503 | 2695 | 2718 | 2536 | 2536 |
| Approach spin rate Sa10 (rpm) | 3738                                | 3749 | 3438 | 3596 | 3604 | 3604 |
| Sd/Sa10                       | 0.68                                | 0.67 | 0.78 | 0.76 | 0.70 | 0.70 |

TABLE 5

|                               |                                     | Golf ball No. |      |      |      |      |
|-------------------------------|-------------------------------------|---------------|------|------|------|------|
|                               |                                     | 3-1           | 3-2  | 3-3  | 3-4  | 3-5  |
| Center                        | Material No.                        | e             | e    | e    | a    | e    |
|                               | Hardness H0 (Shore D)               | 35            | 35   | 35   | 45   | 35   |
|                               | Diameter (mm)                       | 15            | 15   | 15   | 15   | 15   |
| First envelope                | Material No.                        | f             | f    | g    | g    | f    |
| layer                         | Hardness H1 (Shore D)               | 29            | 29   | 25   | 25   | 29   |
| Second envelope               | Thickness (mm)                      | 2.5           | 2.5  | 2.5  | 2.5  | 2.5  |
| layer                         | Material No.                        | C             | C    | D    | D    | C    |
| Third envelope                | Hardness H2 (Shore D)               | 27            | 27   | 19   | 19   | 27   |
| layer                         | Thickness (mm)                      | 2.5           | 2.5  | 2.5  | 2.5  | 2.5  |
| Fourth envelope               | Material No.                        | a             | a    | a    | a    | a    |
| layer                         | Hardness H3 (Shore D)               | 45            | 45   | 45   | 45   | 45   |
| Fifth envelope                | Thickness (mm)                      | 2.5           | 5.0  | 2.5  | 5.0  | 5.0  |
| layer                         | Material No.                        | b             | b    | b    | b    | b    |
| Cover                         | Hardness H4 (Shore D)               | 54            | 54   | 54   | 54   | 54   |
|                               | Thickness (mm)                      | 4.9           | 2.4  | 4.9  | 2.4  | 2.4  |
|                               | Material No.                        | k             | k    | k    | k    | k    |
| First envelope                | Hardness Hn (Shore D)               | 65            | 65   | 65   | 65   | 65   |
| layer                         | Thickness (mm)                      | 1.0           | 1.0  | 1.0  | 1.0  | 1.0  |
| Cover                         | Material No.                        | l             | l    | l    | l    | l    |
|                               | Hardness Hc (Shore D)               | 32            | 32   | 32   | 32   | 32   |
|                               | Thickness (mm)                      | 0.5           | 0.5  | 0.5  | 0.5  | 0.5  |
| Hardness difference (Ho - H2) |                                     | 8             | 8    | 16   | 26   | 8    |
| Hardness difference (H1 - H2) |                                     | 2             | 2    | 6    | 6    | 2    |
| Hardness difference (Hn - H2) |                                     | 30            | 30   | 46   | 46   | 30   |
| Physical properties           | Compression deformation amount (mm) | 2.71          | 2.80 | 2.73 | 2.71 | 2.81 |
|                               | Driver spin rate Sd (rpm)           | 2382          | 2378 | 2326 | 2400 | 2322 |
|                               | Approach spin rate Sa10 (rpm)       | 3797          | 3746 | 3799 | 3801 | 3749 |
|                               | Sd/Sa10                             | 0.63          | 0.63 | 0.61 | 0.63 | 0.62 |

|                               |                                     | Golf ball No. |      |      |      |      |      |
|-------------------------------|-------------------------------------|---------------|------|------|------|------|------|
|                               |                                     | 3-6           | 3-7  | 3-8  | 3-9  | 3-10 | 3-11 |
| Center                        | Material No.                        | f             | f    | f    | g    | a    | f    |
|                               | Hardness H0 (Shore D)               | 29            | 29   | 29   | 25   | 45   | 29   |
|                               | Diameter (mm)                       | 15            | 15   | 20   | 15   | 15   | 15   |
| First envelope                | Material No.                        | a             | a    | a    | a    | g    | g    |
| layer                         | Hardness H1 (Shore D)               | 45            | 45   | 45   | 45   | 25   | 25   |
| Second envelope               | Thickness (mm)                      | 2.5           | 2.5  | 5.0  | 2.5  | 2.5  | 2.5  |
| layer                         | Material No.                        | C             | D    | C    | E    | E    | E    |
| Third envelope                | Hardness H2 (Shore D)               | 27            | 19   | 27   | 45   | 45   | 45   |
| layer                         | Thickness (mm)                      | 2.5           | 2.5  | 2.5  | 7.5  | 7.5  | 7.5  |
| Fourth envelope               | Material No.                        | a             | a    | —    | —    | —    | —    |
| layer                         | Hardness H3 (Shore D)               | 45            | 45   | —    | —    | —    | —    |
| Fifth envelope                | Thickness (mm)                      | 5.0           | 5.0  | —    | —    | —    | —    |
| layer                         | Material No.                        | b             | b    | b    | b    | b    | g    |
| Cover                         | Hardness H4 (Shore D)               | 54            | 54   | 54   | 54   | 54   | 25   |
|                               | Thickness (mm)                      | 2.4           | 2.4  | 2.4  | 2.4  | 2.4  | 2.4  |
|                               | Material No.                        | k             | k    | k    | k    | k    | k    |
| First envelope                | Hardness Hn (Shore D)               | 65            | 65   | 65   | 65   | 65   | 65   |
| layer                         | Thickness (mm)                      | 1.0           | 1.0  | 1.0  | 1.0  | 1.0  | 1.0  |
| Cover                         | Material No.                        | l             | l    | l    | l    | l    | l    |
|                               | Hardness Hc (Shore D)               | 32            | 32   | 32   | 32   | 32   | 32   |
|                               | Thickness (mm)                      | 0.5           | 0.5  | 0.5  | 0.5  | 0.5  | 0.5  |
| Hardness difference (Ho - H2) |                                     | 2             | 10   | 2    | -20  | 0    | -16  |
| Hardness difference (H1 - H2) |                                     | 18            | 26   | 18   | 0    | -20  | -20  |
| Hardness difference (Hn - H2) |                                     | 36            | 36   | 36   | 40   | 20   | 36   |
| Physical properties           | Compression deformation amount (mm) | 2.76          | 2.79 | 3.04 | 2.76 | 2.78 | 2.81 |
|                               | Driver spin rate Sd (rpm)           | 2488          | 2446 | 2566 | 2653 | 2614 | 2479 |
|                               | Approach spin rate Sa10 (rpm)       | 3737          | 3748 | 3590 | 3595 | 3606 | 3558 |
|                               | Sd/Sa10                             | 0.67          | 0.65 | 0.71 | 0.74 | 0.73 | 0.70 |

TABLE 6

|                               |                                     | Golf ball No. |      |      |      |      |      |      |      |
|-------------------------------|-------------------------------------|---------------|------|------|------|------|------|------|------|
|                               |                                     | 4-1           | 4-2  | 4-3  | 4-4  | 4-5  | 4-6  | 4-7  | 4-8  |
| Center                        | Material No.                        | A             | A    | A    | A    | A    | A    | A    | A    |
|                               | Hardness H0 (Shore D)               | 34            | 34   | 34   | 34   | 34   | 34   | 34   | 34   |
|                               | Diameter (mm)                       | 15            | 15   | 15   | 15   | 15   | 15   | 20   | 15   |
| First envelope                | Material No.                        | f             | f    | g    | f    | g    | a    | a    | a    |
|                               | Hardness H1 (Shore D)               | 29            | 29   | 25   | 29   | 25   | 45   | 45   | 45   |
| layer                         | Thickness (mm)                      | 2.5           | 2.5  | 2.5  | 2.5  | 2.5  | 2.5  | 2.5  | 2.5  |
| Second envelope               | Material No.                        | h             | h    | h    | h    | h    | g    | d    | h    |
|                               | Hardness H2 (Shore D)               | 15            | 15   | 15   | 15   | 15   | 25   | 23   | 15   |
| layer                         | Thickness (mm)                      | 2.5           | 2.5  | 2.5  | 2.5  | 2.5  | 2.5  | 2.5  | 2.5  |
| Third envelope                | Material No.                        | a             | a    | a    | a    | a    | a    | a    | a    |
|                               | Hardness H3 (Shore D)               | 45            | 45   | 45   | 45   | 45   | 45   | 45   | 45   |
| layer                         | Thickness (mm)                      | 2.5           | 5.0  | 2.5  | 2.5  | 5.0  | 5.0  | 2.5  | 5.0  |
| Fourth envelope               | Material No.                        | b             | b    | b    | b    | b    | b    | b    | b    |
|                               | Hardness H4 (Shore D)               | 54            | 54   | 54   | 54   | 54   | 54   | 54   | 54   |
| layer                         | Thickness (mm)                      | 4.9           | 2.4  | 4.9  | 4.9  | 2.4  | 2.4  | 2.4  | 2.4  |
| Fifth envelope                | Material No.                        | k             | k    | k    | k    | k    | k    | k    | k    |
|                               | Hardness Hn (Shore D)               | 65            | 65   | 65   | 65   | 65   | 65   | 65   | 65   |
| layer                         | Thickness (mm)                      | 1.0           | 1.0  | 1.0  | 1.0  | 1.0  | 1.0  | 1.0  | 1.0  |
| Cover                         | Material No.                        | 1             | 1    | 1    | 1    | 1    | 1    | 1    | 1    |
|                               | Hardness Hc (Shore D)               | 32            | 32   | 32   | 32   | 32   | 32   | 32   | 32   |
|                               | Thickness (mm)                      | 0.5           | 0.5  | 0.5  | 0.5  | 0.5  | 0.5  | 0.5  | 0.5  |
| Hardness difference (H0 - H2) |                                     | 19            | 19   | 19   | 19   | 19   | 9    | 11   | 19   |
| Hardness difference (H1 - H2) |                                     | 14            | 14   | 10   | 14   | 10   | 20   | 22   | 30   |
| Hardness difference (Hn - H2) |                                     | 50            | 50   | 50   | 50   | 50   | 40   | 42   | 50   |
| Physical properties           | Compression deformation amount (mm) | 2.72          | 2.80 | 2.73 | 2.70 | 2.82 | 2.69 | 2.83 | 2.76 |
|                               | Driver spin rate Sd (rpm)           | 2367          | 2363 | 2311 | 2400 | 2308 | 2639 | 2557 | 2534 |
|                               | Approach spin rate Sa10 (rpm)       | 3799          | 3749 | 3802 | 3749 | 3751 | 3713 | 3510 | 3741 |
|                               | Sd/Sa10                             | 0.62          | 0.63 | 0.61 | 0.65 | 0.62 | 0.71 | 0.73 | 0.68 |

|                               |                                     | Golf ball No. |      |      |      |      |      |
|-------------------------------|-------------------------------------|---------------|------|------|------|------|------|
|                               |                                     | 4-9           | 4-10 | 4-11 | 4-12 | 4-13 | 5-1  |
| Center                        | Material No.                        | A             | A    | A    | A    | A    | A    |
|                               | Hardness H0 (Shore D)               | 34            | 34   | 34   | 34   | 34   | 34   |
|                               | Diameter (mm)                       | 20            | 20   | 15   | 15   | 15   | 15   |
| First envelope                | Material No.                        | a             | a    | a    | g    | g    | B    |
| layer                         | Hardness H1 (Shore D)               | 45            | 45   | 45   | 25   | 25   | 51   |
| Second envelope               | Material No.                        | h             | g    | a    | a    | a    | k    |
| layer                         | Hardness H2 (Shore D)               | 15            | 25   | 45   | 45   | 45   | 65   |
| Third envelope                | Material No.                        | 2.5           | 2.5  | 7.5  | 7.5  | 7.5  | 1    |
| layer                         | Thickness (mm)                      | a             | —    | —    | —    | —    | —    |
| Fourth envelope               | Hardness H3 (Shore D)               | 45            | —    | —    | —    | —    | —    |
| layer                         | Thickness (mm)                      | 2.5           | —    | —    | —    | —    | —    |
| Fifth envelope                | Material No.                        | b             | b    | b    | b    | g    | —    |
| layer                         | Hardness H4 (Shore D)               | 54            | 54   | 54   | 54   | 25   | —    |
| Third envelope                | Material No.                        | 2.4           | 2.4  | 2.4  | 2.4  | 2.4  | —    |
| layer                         | Thickness (mm)                      | Material No.  | b    | b    | b    | g    | —    |
| Fourth envelope               | Hardness H4 (Shore D)               | 54            | 54   | 54   | 54   | 25   | —    |
| layer                         | Thickness (mm)                      | 2.4           | 2.4  | 2.4  | 2.4  | 2.4  | —    |
| Fifth envelope                | Material No.                        | k             | k    | k    | k    | k    | —    |
| layer                         | Hardness Hn (Shore D)               | 65            | 65   | 65   | 65   | 65   | —    |
| Third envelope                | Material No.                        | 1.0           | 1.0  | 1.0  | 1.0  | 1.0  | —    |
| layer                         | Thickness (mm)                      | 1             | 1    | 1    | 1    | 1    | —    |
| Cover                         | Material No.                        | 1             | 1    | 1    | 1    | 1    | 1    |
|                               | Hardness Hc (Shore D)               | 32            | 32   | 32   | 32   | 32   | 32   |
|                               | Thickness (mm)                      | 0.5           | 0.5  | 0.5  | 0.5  | 0.5  | 0.5  |
| Hardness difference (H0 - H2) |                                     | 19            | 9    | -11  | -11  | -11  | —    |
| Hardness difference (H1 - H2) |                                     | 30            | 20   | 0    | -20  | -20  | -14  |
| Hardness difference (Hn - H2) |                                     | 50            | 40   | 20   | 20   | 20   | —    |
| Physical properties           | Compression deformation amount (mm) | 2.90          | 2.87 | 2.59 | 2.64 | 2.87 | 2.60 |
|                               | Driver spin rate Sd (rpm)           | 2511          | 2701 | 2812 | 2630 | 2859 | 2300 |
|                               | Approach spin rate Sa10 (rpm)       | 3462          | 3520 | 3668 | 3676 | 3631 | 3350 |
|                               | Sd/Sa10                             | 0.73          | 0.77 | 0.77 | 0.72 | 0.79 | 0.69 |

## 33

This application is based on Japanese Patent Applications No. 2014-135405 filed on Jun. 30, 2014, and No. 2015-099148 filed on May 14, 2015, the content of which is hereby incorporated by reference.

The invention claimed is:

1. A multi-piece golf ball comprising a spherical center, at least two envelope layers covering the spherical center, and a cover covering the envelope layers, wherein

the envelope layers comprise at least a first envelope layer covering the spherical center, and a second envelope layer covering the first envelope layer,

a material hardness (H0) of the spherical center, a material hardness (H1) of the first envelope layer, and a material hardness (H2) of the second envelope layer satisfy a relationship  $H0 > H1 > H2$ ,

the material hardness (H2) of the second envelope layer is 30 or less in Shore D hardness and lowest among the material hardness of the center and all layers, including all envelope layers, between the center and the cover, a hardness difference (H1-H2) between the material hardness (H1) of the first envelope layer and the material hardness (H2) of the second envelope layer ranges from 1 to 30 in Shore D hardness, and the material hardness (H0) of the spherical center is 35 or less in Shore D hardness.

2. The multi-piece golf ball according to claim 1, wherein a hardness difference (H0-H2) between the material hardness (H2) of the second envelope layer and the material hardness (H0) of the spherical center is 5 or more in Shore D hardness.

3. The multi-piece golf ball according to claim 1, wherein a material hardness (Hc) of the cover ranges from 5 to 55 in Shore D hardness.

4. The multi-piece golf ball according to claim 1, wherein the first envelope layer has a thickness of 15 mm or less, and the second envelope layer has a thickness of 20 mm or less.

5. The multi-piece golf ball according to claim 1, wherein the second envelope layer has a thickness of 2.5 mm or more and 20 mm or less, and the first envelope layer has a thickness of 2.5 mm or less.

6. The multi-piece golf ball according to claim 1, wherein the cover has a thickness of 2 mm or less.

7. The multi-piece golf ball according to claim 1, wherein the spherical center has a diameter ranging from 5 mm to 25 mm.

8. The multi-piece golf ball according to claim 1, wherein a hardness difference (H0-H1) between the material hardness (H0) of the spherical center and the material hardness (H1) of the first envelope layer ranges from 1 to 30 in Shore D hardness.

9. A multi-piece golf ball comprising a spherical center, at least four envelope layers covering the spherical center, and a cover covering the envelope layers,

wherein the envelope layers comprise at least four layers including at least a first envelope layer covering the spherical center, a second envelope layer covering the first envelope layer, and an outermost envelope layer located on the outermost side of the envelope layers;

a material hardness (H0) of the spherical center, a material hardness (H1) of the first envelope layer, and a material hardness (H2) of the second envelope layer satisfy a relationship  $H0 > H1 > H2$ ;

the material hardness (H2) of the second envelope layer is lowest among the material hardness of the center and all layers, including all envelope layers, between the center and the cover;

## 34

a material hardness (Hn) of the outermost envelope layer is highest among the material hardness of the center, the cover and all layers, including all envelope layers, between the center and the cover; and

5 a material hardness (Hx) of an envelope layer disposed between the second envelope layer and the outermost envelope layer, the material hardness (H2) of the second envelope layer, and the material hardness (Hn) of the outermost envelope layer satisfy a relationship  $H2 < Hx < Hn$ .

10 10. The multi-piece golf ball according to claim 9, wherein the material hardness (H2) of the second envelope layer is 30 or less in Shore D hardness.

15 11. The multi-piece golf ball according to claim 9, wherein a hardness difference (Hn-H2) between the material hardness (H2) of the second envelope layer and the material hardness (Hn) of the outermost envelope layer is 25 or more in Shore D hardness.

20 12. The multi-piece golf ball according to claim 9, wherein a hardness difference (H0-H2) between the material hardness (H2) of the second envelope layer and the material hardness (H0) of the spherical center is 5 or more in Shore D hardness.

25 13. The multi-piece golf ball according to claim 9, wherein the material hardness (H0) of the spherical center is 55 or less in Shore D hardness.

14. The multi-piece golf ball according to claim 9, wherein the material hardness (H1) of the first envelope layer ranges from 10 to 50 in Shore D hardness.

30 15. The multi-piece golf ball according to claim 9, wherein the material hardness (Hn) of the outermost envelope layer ranges from 30 to 85 in Shore D hardness.

35 16. The multi-piece golf ball according to claim 9, wherein a material hardness (Hc) of the cover ranges from 5 to 55 in Shore D hardness.

40 17. The multi-piece golf ball according to claim 9, wherein the first envelope layer has a thickness of 15 mm or less, and the material hardness (H0) of the spherical center is 35 or less in Shore D hardness.

45 18. The multi-piece golf ball according to claim 9, wherein the second envelope layer has a thickness of 2.5 mm or more and 20 mm or less, and the first envelope layer has a thickness of 2.5 mm or less.

19. The multi-piece golf ball according to claim 9, wherein the outermost envelope layer has a thickness of 5 mm or less.

50 20. The multi-piece golf ball according to claim 9, wherein the cover has a thickness of 2 mm or less.

21. The multi-piece golf ball according to claim 9, wherein the envelope layer disposed between the second envelope layer and the outermost envelope layer has a thickness of 15 mm or less and is formed from a thermoplastic resin composition containing an ionomer resin as a resin component.

55 22. The multi-piece golf ball according to claim 9, wherein the spherical center has a diameter ranging from 5 mm to 25 mm.

23. The multi-piece golf ball according to claim 9, wherein a hardness difference (H0-H1) between the material hardness (H0) of the spherical center and the material hardness (H1) of the first envelope layer ranges from 1 to 30 in Shore D hardness.

60 24. The multi-piece golf ball according to claim 9, wherein a hardness difference (H1-H2) between the material hardness (H1) of the first envelope layer and the material hardness (H2) of the second envelope layer ranges from 1 to

30 in Shore D hardness, and the material hardness (H0) of the spherical center is 35 or less in Shore D hardness.

**25.** The multi-piece golf ball according to claim 9, wherein a hardness difference (Hn-H0) between the material hardness (Hn) of the outermost envelope layer and the material hardness (H0) of the spherical center ranges from 1 to 70 in Shore D hardness. 5

\* \* \* \* \*